# EUROPEAN PATENT SPECIFICATION

(11) **EP 3 926 030 B1**
(45) Date of publication and mention of the grant of the patent: **28.01.2026**
(21) Application number: 21180346.5
(22) Date of filing: 18.06.2021
(51) Int. Cl.: C11D 17/04, C11D 1/00, C11D 3/22

(54) **WATER-SOLUBLE UNIT DOSE ARTICLE COMPRISING A POLYVINYLALCOHOL FILM AND A CATIONIC POLY ALPHA-1,6-GLUCAN ETHER COMPOUND**
WASSERLÖSLICHER EINHEITSDOSISARTIKEL MIT EINEM POLYVINYLALKOHOLFILM UND EINER KATIONISCHEN POLY-ALPHA-1,6-GLUCANETHERVERBINDUNG
ARTICLE DE DOSE UNITAIRE SOLUBLE DANS L'EAU COMPRENANT UN FILM DE L'ALCOOL POLYVINYLIQUE ET UN COMPOSÉ D'ÉTHER POLY ALPHA-1,6-GLUCANE CATIONIQUE

(30) Priority: 18.06.2020 US 202063040607 P
(43) Date of publication of application: 22.12.2021
(73) Proprietor: The Procter & Gamble Company, Cincinnati, OH 45202 (US)
(72) Inventor: BURKHART, Brandon J., Wilmington, 19805 (US); DEPOOT, Karel Jozef Maria, 1853 Strombeek-Bever (BE); FLITER, Kristine Lynn, Cincinnati, 45202 (US); GAGNON, Michael D., West Grove, 19390 (US); GOOD, David, Cincinnati, 45202 (US); LU, Helen, Wallingford, 19086 (US); QIU, Weiming, Wilmington, 19808 (US); SIVIK, Mark Robert, Cincinnati, 45202 (US); VOLONT, Cedric Joseph, 1853 Strombeek-Bever (BE); WALRAVENS, Wouter, 1853 Strombeek-Bever (BE)
(74) Representative: P&G Patent Belgium UK

(56) References cited:
- EP-A1- 2 399 979
- WO-A1-2018/112187
- US-A1- 2016 311 935

## Description

### FIELD OF THE INVENTION

Water-soluble unit dose articles containing polyvinylalcohol films and a cationic poly alpha-1,6-glucan ether compound, methods of making said water-soluble unit dose articles and methods of using said water-soluble unit dose articles.

### BACKGROUND OF THE INVENTION

Water-soluble unit dose articles are liked by consumers as they offer convenience and ease to the laundry process. Without wishing to be bound by theory, the water-soluble unit dose article comprises a water-soluble film and a unitized dose of a laundry treatment composition which may be with one or more compartments within the unit dose article.

There is a desire for such water-soluble unit dose articles to provide a laundry treatment benefit of both fabric cleaning and fabric enhancing. Fabric enhancing includes benefits such as fabric shape retention, fabric softness and fabric freshness. Fabric freshness is provided by the use of perfumes and perfume delivery technologies.

WO2018/112187 A1 discloses water-soluble unit doses comprising poly alpha-1,6-glucan. US2016/311935 A1 discloses compositions comprising cationic poly alpha-1,6-glucan ether compounds.

EP2399979A discloses a water-soluble unit dose article comprising a polyvinylalcohol based water-soluble film and a cationic polysaccharide polymer. Exemplified in the examples is a cationically modified hydroxethylcellulose, which from WO2004069979 are known to provide both fabric shape retention and fabric softness benefits.

However, an issue observed with such water-soluble unit dose articles, is that both the polyvinylalcohol film and the cationically modified hydroxyethylcellulose have a negative impact on the freshness benefit on fabrics.

Therefore, there is a need in the art for a water-soluble unit dose article comprising a polyvinylalcohol film, that provides fabric shape retention and fabric softness benefits but in which fabric freshness negatives are at least in part mitigated versus water-soluble unit dose articles comprising polyvinylalcohol water-soluble film and cationically modified hydroxyethylcellulose.

It was surprisingly found that the present invention overcame this issue. Without wishing to be bound by theory, it was surprisingly found that a water-soluble unit dose article comprising a polyvinylalcohol water-soluble film and a cationically modified poly alpha-1,6-glucan ether compound provided excellent fabric shape retention and fabric softness whilst exhibiting improved fabric freshness benefit versus a water-soluble unit dose article comprising polyvinylalcohol water-soluble film and cationically modified hydroxyethylcellulose.

### SUMMARY OF THE INVENTION

A first aspect of the present invention is a water-soluble unit dose article comprising a water-soluble film and a liquid laundry treatment composition; wherein the water-soluble film comprises a polyvinylalcohol and is shaped to create an internal compartment, wherein the liquid laundry treatment composition is housed in said internal compartment; and wherein the liquid laundry treatment composition comprises a cationically modified poly alpha-1,6-glucan ether compound, wherein the treatment composition comprises from 0.01% to 10% by weight of the treatment composition, of the cationically modified poly alpha-1,6-glucan ether compound.

A second aspect of the present invention is a process for washing fabrics comprising the steps of diluting a water-soluble unit dose article according to the present invention in water by a factor of between 200 and 3000 fold to create a wash liquor and contacting fabrics to be washed with said wash liquor.

### BRIEF DESCRIPTION OF THE DRAWINGS

FIG.1 is a water-soluble unit dose article according to the present invention.

### DETAILED DESCRIPTION OF THE INVENTION

### Water-soluble unit dose article

A first aspect of the present invention is a water-soluble unit dose article comprising a water-soluble film and a liquid laundry treatment composition. The water-soluble film and the liquid laundry treatment composition are described in more detail below.

The water-soluble unit dose article comprises the water-soluble film shaped such that the unit-dose article comprises at least one internal compartment surrounded by the water-soluble film. The unit dose article may comprise a first water-soluble film and a second water-soluble film sealed to one another such to define the internal compartment. The water-soluble unit dose article is constructed such that the laundry treatment composition does not leak out of the compartment during storage. However, upon addition of the water-soluble unit dose article to water, the water-soluble film dissolves/disintegrates and releases the contents of the internal compartment into the wash liquor.

The compartment should be understood as meaning a closed internal space within the unit dose article, which holds the liquid laundry treatment composition. During manufacture, a first water-soluble film may be shaped to comprise an open compartment into which the liquid laundry treatment composition is added. A second water-soluble film is then laid over the first film in such an orientation as to close the opening of the compartment. The first and second films are then sealed together along a seal region.

The unit dose article may comprise more than one compartment, even at least two compartments, or even at least three compartments, or even at least four compartments. The compartments may be arranged in superposed orientation, i.e. one positioned on top of the other. In such an orientation the unit dose article will comprise at least three films, top, at least one middle and bottom. Alternatively, the compartments may be positioned in a side-by-side orientation, i.e. one orientated next to the other. The compartments may even be orientated in a 'tyre and rim' arrangement, i.e. a first compartment is positioned next to a second compartment, but the first compartment at least partially surrounds the second compartment but does not completely enclose the second compartment. Alternatively, one compartment may be completely enclosed within another compartment.

Wherein the unit dose article comprises at least two compartments, one of the compartments may be smaller than the other compartment. Wherein the unit dose article comprises at least three compartments, two of the compartments may be smaller than the third compartment, and preferably the smaller compartments are superposed on the larger compartment. The superposed compartments preferably are orientated side-by-side.

Wherein the unit dose article comprises at least four compartments, three of the compartments may be smaller than the fourth compartment, and preferably the smaller compartments are superposed on the larger compartment. The superposed compartments preferably are orientated side-by-side.

In a multi-compartment orientation, the detergent composition according to the present invention may be comprised in at least one of the compartments. It may for example be comprised in just one compartment, or may be comprised in two compartments, or even in three compartments, or even in all compartments.

Each compartment may comprise the same or different compositions. The different compositions could all be in the same form, or they may be in different forms.

The water-soluble unit dose article may comprise at least two internal compartments, wherein the liquid laundry detergent composition is comprised in at least one of the compartments, preferably wherein the unit dose article comprises at least three or even four compartments, wherein the liquid laundry treatment composition is comprised in at least one of the compartments.

Preferably, the water-soluble unit dose article comprises between Oppm and 20ppm, preferably between Oppm and 15ppm, more preferably between Oppm and 10ppm, even more preferably between Oppm and 5ppm, even more preferably between Oppm and 1ppm, even more preferably between Oppb and 100ppb, most preferably Oppb dioxane. Those skilled in the art will be aware of known techniques to determine dioxane levels.

FIG.1 discloses a water-soluble unit dose article (1) according to the present invention. The water-soluble unit dose article (1) comprises a first water-soluble film (2) and a second water-soluble film (3) which are sealed together at a seal region (4). The laundry treatment composition (5) is comprised within the water-soluble soluble unit dose article (1).

It was surprisingly found that a water-soluble unit dose article comprising a polyvinylalcohol water-soluble film and a cationically modified poly alpha-1,6-glucan ether compound provided excellent fabric shape retention and fabric softness whilst exhibiting improved fabric freshness benefit versus a water-soluble unit dose article comprising polyvinylalcohol water-soluble film and cationically modified hydroxyethylcellulose. Without wishing to be bound by theory it is believed that the fabric care benefits are driven through the cationically modified polyglucan forming a coacervate phase upon dilution together with the anionic surfactant. The degree of coacervation depends on applied molecule modifications including but not limiting to molecular weight, degree of cationic substitution and degree of hydrophobic modification.

In addition to providing excellent fabric shape retention and fabric softness whilst exhibiting improved fabric freshness benefit, it was surprisingly found that the cationically modified polyglucan also enabled a higher water level within the water-soluble unit dose article without negatively impacting film compatibility. Without wishing to be bound by theory it is believed that the cationically modified polyglucan polymer helps control the amount of free water within the enclosed liquid detergent composition.

### Water-soluble film

The water-soluble film of the present invention is soluble or dispersible in water. The water-soluble film preferably has a thickness of from 20 to 150 micron, preferably 35 to 125 micron, even more preferably 50 to 110 micron, most preferably about 76 micron.

Preferably, the film has a water-solubility of at least 50%, preferably at least 75% or even at least 95%, as measured by the method set out here after using a glass-filter with a maximum pore size of 20 microns:
5 grams ± 0.1 gram of film material is added in a pre-weighed 3L beaker and 2L ± 5ml of distilled water is added. This is stirred vigorously on a magnetic stirrer, Labline model No. 1250 or equivalent and 5 cm magnetic stirrer, set at 600 rpm, for 30 minutes at 30°C. Then, the mixture is filtered through a folded qualitative sintered-glass filter with a pore size as defined above (max. 20 micron). The water is dried off from the collected filtrate by any conventional method, and the weight of the remaining material is determined (which is the dissolved or dispersed fraction). Then, the percentage solubility or dispersability can be calculated.

The water-soluble film material can, for example, be obtained by casting, blow-moulding, extrusion or blown extrusion of the polymeric material, as known in the art.

The water-soluble film comprises polyvinylalcohol. The polyvinylalcohol may be present between 50% and 95%, preferably between 55% and 90%, more preferably between 60% and 80% by weight of the water soluble film. Preferably, the water-soluble film comprises polyvinyl alcohol homopolymer or polyvinylalcohol copolymer, preferably a blend of polyvinylalcohol homopolymers and/or anionic polyvinylalcohol copolymers preferably selected from sulphonated and carboxylated anionic polyvinylalcohol copolymers especially carboxylated anionic polyvinylalcohol copolymers, most preferably a blend of a polyvinylalcohol homopolymer and a carboxylated anionic polyvinylalcohol copolymer. Without wishing to be bound by theory, the term "homopolymer" generally includes polymers having a single type of monomeric repeating unit (e.g., a polymeric chain consisting of or consisting essentially of a single monomeric repeating unit). For the particular case of polyvinylalcohol, the term "homopolymer" further includes copolymers having a distribution of vinyl alcohol monomer units and optionally vinyl acetate monomer units, depending on the degree of hydrolysis (e.g., a polymeric chain consisting of or consisting essentially of vinyl alcohol and vinyl acetate monomer units). In the limiting case of 100% hydrolysis, a polyvinylalcohol homopolymer can include a true homopolymer having only vinyl alcohol units. Without wishing to be bound by theory, the term "copolymer" generally includes polymers having two or more types of monomeric repeating units (e.g., a polymeric chain consisting of or consisting essentially of two or more different monomeric repeating units, whether as random copolymers, block copolymers, etc.). For the particular case of polyvinylalcohol, the term "copolymer" (or "polyvinylalcohol copolymer") further includes copolymers having a distribution of vinyl alcohol monomer units and vinyl acetate monomer units, depending on the degree of hydrolysis, as well as at least one other type of monomeric repeating unit (e.g., a ter- (or higher) polymeric chain consisting of or consisting essentially of vinyl alcohol monomer units, vinyl acetate monomer units, and one or more other monomer units, for example anionic monomer units). In the limiting case of 100% hydrolysis, a polyvinylalcohol copolymer can include a copolymer having vinyl alcohol units and one or more other monomer units, but no vinyl acetate units. Without wishing to be bound by theory, the term "anionic copolymer" includes copolymers having an anionic monomer unit comprising an anionic moiety. General classes of anionic monomer units which can be used for the anionic polyvinyl alcohol co-polymer include the vinyl polymerization units corresponding to monocarboxylic acid vinyl monomers, their esters and anhydrides, dicarboxylic monomers having a polymerizable double bond, their esters and anhydrides, vinyl sulfonic acid monomers, and alkali metal salts of any of the foregoing. Examples of suitable anionic monomer units include the vinyl polymerization units corresponding to vinyl anionic monomers including vinyl acetic acid, maleic acid, monoalkyl maleate, dialkyl maleate, monomethyl maleate, dimethyl maleate, maleic anyhydride, fumaric acid, monoalkyl fumarate, dialkyl fumarate, monomethyl fumarate, dimethyl fumarate, fumaric anyhydride, itaconic acid, monomethyl itaconate, dimethyl itaconate, itaconic anhydride, vinyl sulfonic acid, allyl sulfonic acid, ethylene sulfonic acid, 2-acrylamido-1-methylpropanesulfonic acid, 2-acrylamido-2-methylpropanesulfonic acid, 2-methylacrylamido-2-methylpropanesulfonic acid, 2-sufoethyl acrylate, alkali metal salts of the foregoing (e.g., sodium, potassium, or other alkali metal salts), esters of the foregoing (e.g., methyl, ethyl, or other C1-C4 or C6 alkyl esters), and combinations thereof (e.g., multiple types of anionic monomers or equivalent forms of the same anionic monomer). The anionic monomer may be one or more acrylamido methylpropanesulfonic acids (e.g., 2-acrylamido-1-methylpropanesulfonic acid, 2-acrylamido-2-methylpropanesulfonic acid, 2-methylacrylamido-2-methylpropanesulfonic acid), alkali metal salts thereof (e.g., sodium salts), and combinations thereof. Preferably, the anionic moiety of the first anionic monomer unit is selected from a sulphonate, a carboxylate, or a mixture thereof, more preferably a carboxylate, most preferably an acrylate, a methacrylate, a maleate, or a mixture thereof. Preferably, the anionic monomer unit is present in the anionic polyvinyl alcohol copolymer in an average amount in a range of between 1 mol.% and 10 mol.%, preferably between 2 mol.% and 5 mol.%. Preferably, the polyvinyl alcohol, and/or in case of polyvinylalcohol blends the individual polyvinylalcohol polymers, have an average viscosity (µ1) in a range of between 4 mPa.s and 30 mPa.s, preferably between 10mPa.s and 25 mPa.s, measured as a 4% polyvinyl alcohol copolymer solution in demineralized water at 20 degrees C. The viscosity of a polyvinyl alcohol polymer is determined by measuring a freshly made solution using a Brookfield LV type viscometer with UL adapter as described in British Standard EN ISO 15023-2:2006 Annex E Brookfield Test method. It is international practice to state the viscosity of 4% aqueous polyvinyl alcohol solutions at 20 °C. It is well known in the art that the viscosity of an aqueous water-soluble polymer solution (polyvinylalcohol or otherwise) is correlated with the weight-average molecular weight of the same polymer, and often the viscosity is used as a proxy for weight-average molecular weight. Thus, the weight-average molecular weight of the polyvinylalcohol can be in a range of 30,000 to 175,000, or 30,000 to 100,000, or 55,000 to 80,000. Preferably, the polyvinyl alcohol, and/or in case of polyvinylalcohol blends the individual polyvinylalcohol polymers, have an average degree of hydrolysis in a range of between 75% and 99%, preferably between 80% and 95%, most preferably between 85% and 95%. A suitable test method to measure the degree of hydrolysis is as according to standard method JIS K6726.

Most preferably the polyvinylalcohol is a blend of a polyvinylalcohol homopolymer and a carboxylated anionic polyvinylalcohol copolymer, wherein the homopolymer and the anionic copolymer are present in a relative weight ratio of 90/10 to 10/90, preferably 80/20 to 20/80, more preferably 70/30 to 50/50.

Preferably, the water-soluble film comprises a non-aqueous plasticizer. Preferably, the non-aqueous plasticizer is selected from polyols, sugar alcohols, and mixtures thereof. Suitable polyols include polyols selected from the group consisting of glycerol, diglycerin, ethylene glycol, diethylene glycol, triethyleneglycol, tetraethylene glycol, polyethylene glycols up to 400 MW, neopentyl glycol, 1,2-propylene glycol, 1,3-propanediol, dipropylene glycol, polypropylene glycol, 2-methyl-1,3-propanediol, trimethylolpropane and polyether polyols, or a mixture thereof. Suitable sugar alcohols include sugar alcohols selected from the group consisting of isomalt, maltitol, sorbitol, xylitol, erythritol, adonitol, dulcitol, pentaerythritol and mannitol, or a mixture thereof. More preferably the non-aqueous plasticizer is selected from glycerol, 1,2-propanediol, dipropylene glycol, 2-methyl-1,3-propanediol, trimethylolpropane, triethyleneglycol, polyethyleneglycol, sorbitol, or a mixture thereof, most preferably selected from glycerol, sorbitol, trimethylolpropane, dipropylene glycol, and mixtures thereof. One particularly suitable plasticizer system includes a blend of glycerol, sorbitol and trimethylol propane. Another particularly suitable plasticizer system includes a blend of glycerin, dipropylene glycol, and sorbitol. Preferably, the film comprises between 5% and 50%, preferably between 10% and 40%, more preferably between 20% and 30% by weight of the film of the non-aqueous plasticizer.

Preferably, the water-soluble film comprises a surfactant. Preferably, the water-soluble film comprises a surfactant in an amount between 0.1% and 2.5%, preferably between 1% and 2% by weight of the water-soluble film. Suitable surfactants can include the nonionic, cationic, anionic and zwitterionic classes. Suitable surfactants include, but are not limited to, polyoxyethylenated polyoxypropylene glycols, alcohol ethoxylates, alkylphenol ethoxylates, tertiary acetylenic glycols and alkanolamides (nonionics), polyoxyethylenated amines, quaternary ammonium salts and quaternized polyoxyethylenated amines (cationics), and amine oxides, N-alkylbetaines and sulfobetaines (zwitterionics). Other suitable surfactants include dioctyl sodium sulfosuccinate, lactylated fatty acid esters of glycerol and propylene glycol, lactylic esters of fatty acids, sodium alkyl sulfates, polysorbate 20, polysorbate 60, polysorbate 65, polysorbate 80, lecithin, acetylated fatty acid esters of glycerol and propylene glycol, and acetylated esters of fatty acids, and combinations thereof.

Preferably the water-soluble film according to the invention comprises lubricants / release agents. Suitable lubricants/release agents can include, but are not limited to, fatty acids and their salts, fatty alcohols, fatty esters, fatty amines, fatty amine acetates and fatty amides. Preferred lubricants/release agents are fatty acids, fatty acid salts, and fatty amine acetates. the amount of lubricant/release agent in the water-soluble film is in a range of from 0.02% to 1.5%, preferably from 0.1% to 1% by weight of the water-soluble film.

Preferably, the water-soluble film comprises fillers, extenders, antiblocking agents, detackifying agents or a mixture thereof. Suitable fillers, extenders, antiblocking agents, detackifying agents or a mixture thereof include, but are not limited to, starches, modified starches, crosslinked polyvinylpyrrolidone, crosslinked cellulose, microcrystalline cellulose, silica, metallic oxides, calcium carbonate, talc and mica. Preferred materials are starches, modified starches and silica. Preferably, the amount of filler, extender, antiblocking agent, detackifying agent or mixture thereof in the water-soluble film is in a range of from 0.1% to 25%, preferably from 1% to 10%, more preferably from 2% to 8%, most preferably from 3% to 5% by weight of the water-soluble film. In the absence of starch, one preferred range for a suitable filler, extender, antiblocking agent, detackifying agent or mixture thereof is from 0.1% to 1%, preferably 4%, more preferably 6%, even more preferably from 1% to 4%, most preferably from 1% to 2.5%, by weight of the water-soluble film.

Preferably the water-soluble film according to the invention has a residual moisture content of at least 4%, more preferably in a range of from 4% to 15%, even more preferably of from 5% to 10% by weight of the water-soluble film as measured by Karl Fischer titration.

Preferred films exhibit good dissolution in cold water, meaning unheated distilled water. Preferably such films exhibit good dissolution at temperatures of 24°C, even more preferably at 10°C. By good dissolution it is meant that the film exhibits water-solubility of at least 50%, preferably at least 75% or even at least 95%, as measured by the method set out here after using a glass-filter with a maximum pore size of 20 microns, described above.

Preferred films include those supplied by Monosol under the trade references M8630, M8900, M8779, M83 10.

The film may be opaque, transparent or translucent. The film may comprise a printed area. The area of print may be achieved using standard techniques, such as flexographic printing or inkjet printing. Preferably, the ink used in the printed area comprises between Oppm and 20ppm, preferably between Oppm and 15ppm, more preferably between Oppm and 10ppm, even more preferably between Oppm and 5ppm, even more preferably between Oppm and 1ppm, even more preferably between Oppb and 100ppb, most preferably Oppb dioxane. Those skilled in the art will be aware of known methods and techniques to determine the dioxane level within the ink formulations.

The film may comprise an aversive agent, for example a bittering agent. Suitable bittering agents include, but are not limited to, naringin, sucrose octaacetate, quinine hydrochloride, denatonium benzoate, or mixtures thereof. Any suitable level of aversive agent may be used in the film. Suitable levels include, but are not limited to, 1 to 5000ppm, or even 100 to 2500ppm, or even 250 to 2000rpm.

Preferably, the water-soluble film or water-soluble unit dose article or both are coated in a lubricating agent, preferably, wherein the lubricating agent is selected from talc, zinc oxide, silicas, siloxanes, zeolites, silicic acid, alumina, sodium sulphate, potassium sulphate, calcium carbonate, magnesium carbonate, sodium citrate, sodium tripolyphosphate, potassium citrate, potassium tripolyphosphate, calcium stearate, zinc stearate, magnesium stearate, starch, modified starches, clay, kaolin, gypsum, cyclodextrins or mixtures thereof.

Preferably, the water-soluble film, and each individual component thereof, independently comprises between Oppm and 20ppm, preferably between Oppm and 15ppm, more preferably between Oppm and 10ppm, even more preferably between Oppm and 5ppm, even more preferably between Oppm and 1ppm, even more preferably between Oppb and 100ppb, most preferably Oppb dioxane. Those skilled in the art will be aware of known methods and techniques to determine the dioxane level within water-soluble films and ingredients thereof.

### Liquid laundry treatment composition

The present invention is to a liquid laundry treatment composition. The term 'liquid laundry treatment composition' refers to any laundry treatment composition comprising a liquid capable of wetting and treating a fabric, and includes, but is not limited to, liquids, gels, pastes, dispersions and the like. The liquid composition can include solids or gases in suitably subdivided form, but the liquid composition excludes forms which are non-fluid overall, such as tablets or granules.

The liquid laundry treatment composition comprises a cationically modified poly alpha-1,6-glucan ether compound. The poly alpha-1,6-glucan ether compound is described in more detail below.

Preferably, the liquid laundry treatment composition according to the invention, or any ingredients therein, each individually comprise between Oppm and 20ppm, preferably between Oppm and 15ppm, more preferably between Oppm and 10ppm, even more preferably between Oppm and 5ppm, even more preferably between Oppm and 1ppm, even more preferably between Oppm and100ppb dioxane, most preferably Oppm dioxane. Those skilled in the art will be aware of known methods and techniques to determine the dioxane level within the liquid detergent compositions

Preferably, the liquid laundry treatment composition comprises between 1% and 20%, preferably between 5% and 15% by weight of the liquid laundry detergent composition of water.

Preferably, the liquid laundry treatment composition comprises a non-soap surfactant, wherein the non-soap surfactant preferably comprises anionic surfactant, non-ionic surfactant, cationic surfactant, amphoteric surfactant, zwitterionic surfactant, or a mixture thereof, preferably wherein the liquid treatment composition comprises between 20% and 60%, preferably between 25% and 55%, more preferably between 30% and 50% by weight of the liquid laundry treatment composition of the non-soap surfactant.

Preferably the non-soap surfactant comprises a non-soap anionic surfactant. Preferably the laundry treatment composition comprises between 10% and 50%, between 15% and 45%, between 20% and 40%, or between 30% and 40% by weight of the laundry treatment composition of the non-soap anionic surfactant.

Preferably, the non-soap anionic surfactant comprises linear alkylbenzene sulphonate. Preferably, the linear alkylbenzene sulphonate comprises C₁₀-C₁₆ alkyl benzene sulfonate, C₁₁-C₁₄ alkyl benzene sulphonate or a mixture thereof. Preferably, the alkylbenzene sulphonate is an amine neutralized alkylbenzene sulphonate, an alkali metal neutralized alkylbenzene sulphonate or a mixture thereof. The amine is preferably selected from monoethanolamine, triethanolamine or mixtures thereof. The alkali metal is preferably selected from sodium, potassium, magnesium or a mixture thereof. Preferably, the liquid laundry treatment composition comprises between 5% and 40%, preferably between 10% and 35%, more preferably between 15% and 30% by weight of the liquid laundry treatment composition of the linear alkylbenzene sulphonate anionic surfactant.

Preferably, the non-soap anionic surfactant comprises an alkyl sulphate anionic surfactant wherein the alkyl sulphate anionic surfactant is selected from alkyl sulphate, an alkoxylated alkyl sulphate or a mixture thereof. The alkyl sulphate anionic surfactant may be a primary or a secondary alkyl sulphate anionic surfactant, or a mixture thereof, preferably a primary alkyl sulphate anionic surfactant. Preferably, the alkoxylated alkyl sulphate comprises ethoxylated alkyl sulphate, propoxylated alkyl sulphate, a mixed ethoxylated/propoxylated alkyl sulphate, or a mixture thereof, more preferably an ethoxylated alkyl sulphate. Preferably, the ethoxylated alkyl sulphate has an average degree of ethoxylation of between 0.1 to 5, preferably between 0.5 and 3. Preferably, the ethoxylated alkyl sulphate has an average alkyl chain length of between 8 and 18, more preferably between 10 and 16, most preferably between 12 and 15. Preferably, the alkyl chain of the alkyl sulphate anionic surfactant is linear, branched or a mixture thereof. Preferably, the branched alkyl sulphate anionic surfactant is a branched primary alkyl sulphate, a branched secondary alkyl sulphate, or a mixture thereof, preferably a branched primary alkyl sulphate, wherein the branching preferably is in the 2-position, or alternatively might be present further down the alkyl chain, or could be multi-branched with branches spread over the alkyl chain. The weight average degree of branching of alkyl sulphate anionic surfactant may be from 0% to 100% preferably from 0% to 95%, more preferably from 0% to 60%, most preferably from 0% to 20%. Alternatively, the weight average degree of branching of alkyl sulphate anionic surfactant may be from 70% to 100%, preferably from 80% to 90%. Preferably, the alkyl chain is selected from naturally derived material, synthetically derived material or mixtures thereof. Preferably, the synthetically derived material comprises oxo-synthesized material, Ziegler-synthesized material, Guerbet-synthesized material, Fischer-Tropsch - synthesized material, iso-alkyl synthesized material, or mixtures thereof, preferably oxo-synthesized material. Preferably, the liquid laundry detergent composition comprises between 1% and 35%, preferably between 3% and 30%, more preferably between 6% and 20% by weight of the liquid laundry treatment composition of the alkyl sulphate anionic surfactant.

Preferably, the non-soap anionic surfactant comprises linear alkyl benzene sulphonate and an alkoxylated alkyl sulphate and wherein the weight ratio of linear alkylbenzene sulphonate to alkoxylated alkyl sulphate is from 1:2 to 9:1, preferably from 1:1 to 7:1, more preferably from 1:1 to 5:1, most preferably from 1:1 to 4:1. Without wishing to be bound by theory formulating these anionic surfactant ratios provide the benefit of providing excellent stain removal and cleaning across a broad range of stains.

Preferably, the non-soap surfactant comprises a non-ionic surfactant, wherein the non-ionic surfactant preferably comprises an alkoxylated alcohol, wherein the alkoxylated alcohol is derived from a synthetical alcohol, a natural alcohol or a mixture thereof. The alkoxylated alcohol can be a primary alkoxylated alcohol, a secondary alkoxylated alcohol, or a mixture thereof, preferably a primary alkoxylated alcohol. Preferably, the alkoxylated alcohol comprises ethoxylated alcohol, propoxylated alcohol, a mixed ethoxylated/propoxylated alcohol, or a mixture thereof, more preferably an ethoxylated alcohol. Alternatively, the alkoxylated alcohol might also include higher alkoxy groups such as butoxy groups. When mixed alkoxy groups, the alkoxy groups can be randomnly ordered or present in blocks, preferably are present in blocks. For example, mixed ethoxy (EO)/propoxy (PO) groups might be ordered in EO/PO blocks, PO/EO blocks, EO/PO/EO blocks or PO/EO/PO blocks. Preferably, the ethoxylated alcohol has an average degree of ethoxylation of between 0.1 to 20, preferably between 5 and 15, most preferably between 6 and 10. If propoxylation is present, preferably the average degree of propoxylation is between 0.1 to 25, more preferably between 2 and 20, most preferably between 5 and 10. Preferably, the alkoxylated preferably ethoxylated alcohol has an average alkyl chain length of between 8 and 18, more preferably between 10 and 16, most preferably 12 and 15. Preferably, the alkyl chain of the alkoxylated alcohol is linear, branched or a mixture thereof, wherein the branched alkyloxylated alcohol is a branched primary alkoxylated alcohol, a branched secondary alkoxylated alcohol, or a mixture thereof, preferably a branched primary alkoxylated alcohol. Preferably, the weight average degree of branching of the alkoxylated alcohol is from 0% to 100% preferably from 0% to 95%, more preferably 0% to 60%, most preferably from 0% to 20%. The branching can be on the 2-alkyl position, or alternatively further down the alkyl chain, or can be multi-branched with individual branches spread over the alkyl chain. Preferably, the synthetically derived material comprises oxo-synthesized material, Ziegler-synthesized material, Guerbet-synthesized material, Fischer-Tropsch - synthesized material, iso-alkyl branched materials, or mixtures thereof, preferably oxo-synthesised material. Preferably, the liquid laundry detergent composition comprises between 0.5% and 20%, preferably between 1% and 15%, more preferably between 3% and 12% by weight of the liquid laundry detergent composition of the non-ionic surfactant, preferably wherein the nonionic surfactant consists of the alkoxylated alcohol. Without wishing to be bound by theory, non-ionic surfactants, especially alkoxylated alcohol non-ionic surfactants provide the benefit of excellent body soil cleaning and soil suspension. Preferably the laundry treatment composition comprises between 0.01% and 10%, between 0.01% and 8%, between 0.1% and 6%, or between 0.15% and 5% by weight of the liquid laundry treatment composition of a non-ionic surfactant.

Preferably, the weight ratio of non-soap anionic surfactant to nonionic surfactant is from 1:1 to 20:1, from 1.5:1 to 17.5:1, from 2:1 to 15:1, or from 2.5:1 to 13:1.

Preferably, the liquid laundry treatment composition comprises a fatty acid, preferably a neutralized fatty acid soap, more preferably. Preferably, the liquid laundry treatment composition comprises between 1.5% and 20%, more preferably between 2% and 15%, even more preferably between 3% and 10%, or most preferably between 4% and 8% by weight of the liquid treatment composition of fatty acid. Preferably, the fatty acid may be branched or linear, alkoxylated or non-alkoxylated and preferably is selected from palm kernel fatty acid, coconut fatty acid, rapeseed fatty acid, neutralized palm kernel fatty acid, neutralized coconut fatty acid, neutralized rapeseed fatty acid, or mixture thereof, most preferably a neutralized palm kernel fatty acid. Preferably, the fatty acid soap is neutralised with an alkali metal, an amine, or a mixture thereof. Preferably, the amine is selected from monoethanolamine, triethanolamine or mixtures thereof and the alkali metal is selected from sodium, potassium, magnesium or a mixture thereof. Without wishing to be bound by theory, fatty acid, preferably neutralized fatty acids, provide the benefit of protecting anionic non-soap surfactant from precipitation. Furthermore, they provide the benefit of clay soil removal and body soil cleaning on fabrics.

Preferably, the liquid laundry treatment composition comprises perfume raw material. The perfume raw material may comprise a perfume raw material selected from the group consisting of perfume raw materials having a boiling point (B.P.) lower than about 250°C and a ClogP lower than about 3, perfume raw materials having a B.P. of greater than about 250°C and a ClogP of greater than about 3, perfume raw materials having a B.P. of greater than about 250°C and a ClogP lower than about 3, perfume raw materials having a B.P. lower than about 250°C and a ClogP greater than about 3 and mixtures thereof. Perfume raw materials having a boiling point B.P. lower than about 250°C and a ClogP lower than about 3 are known as Quadrant I perfume raw materials. Quadrant 1 perfume raw materials are preferably limited to less than 30% of the perfume comprosition. Perfume raw materials having a B.P. of greater than about 250°C and a ClogP of greater than about 3 are known as Quadrant IV perfume raw materials, perfume raw materials having a B.P. of greater than about 250°C and a ClogP lower than about 3 are known as Quadrant II perfume raw materials, perfume raw materials having a B.P. lower than about 250°C and a ClogP greater than about 3 are known as a Quadrant III perfume raw materials.

Preferred perfume raw material classes include ketones and aldehydes. Those skilled in the art will know how to formulate an appropriate perfume raw material.

Preferably, the liquid laundry treatment composition comprises one or more adjunct ingredients, wherein the adjunct ingredient is selected from an amphiphilic graft polymer, ethoxylated polyethyleneimine, amphiphilic alkoxylated polyalkyleneimine, an ethyleneoxide (EO) - propyleneoxide (PO) - ethyleneoxide (EO) triblock co-polymer, zwitterionic polyamine, polyester terephthalate, organic solvents, aesthetic dyes, hueing dyes, opacifiers such as those commercially available under the Acusol tradename, brighteners including FWA49, FWA15 and FWA36, dye transfer inhibitors including PVNO, PVP and PVPVI dye transfer inhibitors, builders including citric acid, chelants, enzymes, perfume capsules, preservatives, antioxidants including sulfite salts such as potassium sulphite or potassium bisulphite salts and those commercially available under the Ralox brandname, antibacterial and anti-viral agents including 4.4'-dichloro 2-hydroxydiphenyl ether such as Tinosan HP100 available from the BASF company, anti-mite actives such as benzyl benzoate, structuring agents including hydrogenated castor oil, silicone based anti-foam materials, electrolytes including inorganic electrolytes such as sodium chloride, potassium chloride, magnesium chloride, and calcium chloride, and related sodium, potassium, magnesium and calcium sulphate salts, as well as organic electrolytes such as sodium, potassium, magnesium and calcium salts of carbonate, bicarbonate, carboxylates such as formate, citrate and acetate. pH trimming agents including sodium hydroxide, hydrogen chloride and alkanolamines including monoethanolamine, diethanolamine and triethanolamine, or a mixture thereof. Preferably, the organic solvent is selected from alcohols including ethanol, propanol, isopropanol, and mixtures thereof, polyols including sugar alcohols, glycols, glycol ethers, and mixtures thereof, preferably polyethylene glycol especially low molecular weight polyethyleneglycols such as PEG 200 and PEG 400, diethylene glycol, glycerol, 1,2-propanediol, polypropylene glycol including dipropyleneglycol and tripropyleneglycol and low molecular weight polypropyeleneglycols such as PPG400, sorbitol, or a mixture thereof. Preferably, the chelant is selected from EDDS, HEDP, GLDA, DTPA, DTPMP, DETA, or mixtures thereof. Preferably, the enzyme is selected from protease, amylase, cellulase, mannanase, lipase, xyloglucanase, pectate lyase, nuclease enzyme, or a mixture thereof.

Preferably the liquid laundry treatment composition has a pH between 6 and 10, between 6.5 and 8.9, or between 7 and 8, wherein the pH of the liquid laundry treatment composition is measured as a 10% product concentration in demineralized water at 20°C.

The liquid laundry treatment composition may be Newtonian or non-Newtonian. Preferably, the liquid laundry treatment composition is non-Newtonian. Without wishing to be bound by theory, a non-Newtonian liquid has properties that differ from those of a Newtonian liquid, more specifically, the viscosity of non-Newtonian liquids is dependent on shear rate, while a Newtonian liquid has a constant viscosity independent of the applied shear rate. The decreased viscosity upon shear application for non-Newtonian liquids is thought to further facilitate liquid detergent dissolution. The liquid laundry treatment composition described herein can have any suitable viscosity depending on factors such as formulated ingredients and purpose of the composition.

### Cationically modified poly alpha-1,6-glucan ether compound

The liquid laundry treatment composition comprises a cationically modified poly alpha-1,6-glucan ether compound. Preferably, the cationically modified poly alpha-1,6-glucan ether compound comprises a poly alpha-1,6-glucan substituted with at least one positively charged organic group, wherein the poly alpha-1,6-glucan comprises a backbone of glucose monomer units wherein at least 65% of the glucose monomer units are linked via alpha-1,6-glycosidic linkages, and wherein the poly alpha-1,6-glucan ether compound has a degree of substitution of about 0.001 to about 3; and is characterised by at least one of the following i-iv;
i) a weight average degree of polymerization of at least 5;
ii) a weight average molecular weight of from about 1000 to about 500,000 daltons;
iii) been derived from a poly alpha-1,6-glucan having a weight average molecular weight of from about 900 to about 450,000 daltons, determined prior to substitution with the least one positively charged organic group;
iv) a mixture thereof.

As used herein, the term "polysaccharide" means a polymeric carbohydrate molecule composed of long chains of monosaccharide units bound together by glycosidic linkages and on hydrolysis gives the constituent monosaccharides or oligosaccharides.

The term "polysaccharide derivative" as used herein means a chemically modified polysaccharide in which at least some of the hydroxyl groups of the glucose monomer units have been replaced with one or more ether groups. As used herein, the term "polysaccharide derivative" is used interchangeably with "poly alpha-1,6-glucan ether" and "poly alpha-1,6-glucan ether compound".

The term "hydrophobic" refers to a molecule or substituent which is nonpolar and has little or no affinity for water, and which tends to repel water.

The term "hydrophilic" refers to a molecule or a substituent which is polar and has affinity to interact with polar solvents, in particular with water, or with other polar groups. A hydrophilic molecule or substituent tends to attract water.

The "molecular weight" of a poly alpha-1,6-glucan or poly alpha-1,6-glucan ether can be represented as statistically averaged molecular mass distribution, i.e. as number-average molecular weight (Mₙ) or as weight-average molecular weight (M_{w}), both of which are generally given in units of Daltons (Da), i.e. in grams/mole. Alternatively, molecular weight can be represented as DPw (weight average degree of polymerization) or DPn (number average degree of polymerization). Various means are known in the art for calculating these molecular weights from techniques such as high-pressure liquid chromatography (HPLC), size exclusion chromatography (SEC), gel permeation chromatography (GPC), and gel filtration chromatography (GFC).

As used herein, "weight average molecular weight" or "M_{w}" is calculated as

M_{w} = ΣNᵢMᵢ² / ΣNᵢMᵢ; where Mᵢ is the molecular weight of an individual chain i and Nᵢ is the number of chains of that molecular weight. In addition to using SEC, the weight average molecular weight can be determined by other techniques such as static light scattering, mass spectrometry especially MALDI-TOF (matrix-assisted laser desorption/ionization time-of-flight), small angle X-ray or neutron scattering, and ultracentrifugation.

As used herein, "number average molecular weight" or "Mₙ" refers to the statistical average molecular weight of all the polymer chains in a sample. The number average molecular weight is calculated as Mₙ = ΣNᵢMᵢ / ΣNᵢ where Mᵢ is the molecular weight of a chain i and Nᵢ is the number of chains of that molecular weight. In addition to using SEC, the number average molecular weight of a polymer can be determined by various colligative methods such as vapor pressure osmometry or end-group determination by spectroscopic methods such as proton NMR, FTIR, or UV-vis.

As used herein, number average degree of polymerization (DPn) and weight average degree of polymerization (DPw) are calculated from the corresponding average molecular weights Mw or Mn by dividing by the molar mass of one monomer unit M₁. In the case of unsubstituted glucan polymer, M₁ = 162. In the case of a substituted glucan polymer, M₁ = 162 + M_{f} x DoS, where M_{f} is the molar mass of the substituent group and DoS is the degree of substitution with respect to that substituent group (average number of substituted groups per one glucose unit).

Glucose carbon positions 1, 2, 3, 4, 5 and 6 as referred to herein are as known in the art and depicted in Structure I:

The terms "glycosidic linkage" and "glycosidic bond" are used interchangeably herein and refer to the type of covalent bond that joins a carbohydrate (sugar) molecule to another group such as another carbohydrate. The term "alpha-1,6-glucosidic linkage" as used herein refers to the covalent bond that joins alpha-D-glucose molecules to each other through carbons 1 and 6 on adjacent alpha-D-glucose rings. The term "alpha-1,3-glucosidic linkage" as used herein refers to the covalent bond that joins alpha-D-glucose molecules to each other through carbons 1 and 3 on adjacent alpha-D-glucose rings. The term "alpha-1,2-glucosidic linkage" as used herein refers to the covalent bond that joins alpha-D-glucose molecules to each other through carbons 1 and 2 on adjacent alpha-D-glucose rings. The term "alpha-1,4-glucosidic linkage" as used herein refers to the covalent bond that joins alpha-D-glucose molecules to each other through carbons 1 and 4 on adjacent alpha-D-glucose rings. Herein, "alpha-D-glucose" will be referred to as "glucose".

The glycosidic linkage profile of a glucan, dextran, substituted glucan, or substituted dextran can be determined using any method known in the art. For example, a linkage profile can be determined using methods that use nuclear magnetic resonance (NMR) spectroscopy (e.g., ¹³C NMR or ¹H NMR). These and other methods that can be used are disclosed in Food Carbohydrates: Chemistry, Physical Properties, and Applications (S. W. Cui, Ed., Chapter 3, S. W. Cui, Structural Analysis of Polysaccharides, Taylor & Francis Group LLC, Boca Raton, FL, 2005), which is incorporated herein by reference.

The structure, molecular weight, and degree of substitution of a polysaccharide or polysaccharide derivative can be confirmed using various physiochemical analyses known in the art such as NMR spectroscopy and size exclusion chromatography (SEC).

The term "alkyl group", as used herein, refers to linear, branched, aralkyl (such as benzyl), or cyclic ("cycloalkyl") hydrocarbon groups containing no unsaturation. As used herein, the term "alkyl group" encompasses substituted alkyls, for example alkyl groups substituted with at least one hydroxyalkyl group or dihydroxy alkyl group, as well as alkyl groups containing one or more heteroatoms such as oxygen, sulfur, and/or nitrogen within the hydrocarbon chain.

As used herein, the term "aryl" means an aromatic carbocyclic group having a single ring (e.g., phenyl), multiple rings (e.g., biphenyl), or multiple condensed rings in which at least one is aromatic, (e.g., 1,2,3,4-tetrahydronaphthyl, naphthyl, anthryl, or phenanthryl), which is optionally mono-, di-, or trisubstituted with alkyl groups. By aryl is also meant heteroaryl groups where heteroaryl is defined as 5-, 6-, or 7-membered aromatic ring systems having at least one hetero atom selected from the group consisting of nitrogen, oxygen and sulfur. Examples of heteroaryl groups include pyridyl, pyrimidinyl, pyrrolyl, pyrazolyl, pyrazinyl, pyridazinyl, oxazolyl, furanyl, imidazole, quinolinyl, isoquinolinyl, thiazolyl, and thienyl, which can optionally be substituted with alkyl groups.

The poly alpha-1,6-glucan ether compound comprises a poly alpha-1,6-glucan substituted with at least one positively charged organic group, where the poly alpha-1,6-glucan comprises a backbone of glucose monomer units, where at least 65% of the glucose monomer units are linked via alpha-1,6-glycosidic linkages. The poly alpha-1,6-glucan ether compound may be characterized by (a) a weight average degree of polymerization of at least 5; (b) a weight average molecular weight of from about 1000 to about 500,000 daltons; and/or (c) having been derived from a poly alpha-1,6-glucan having a weight average molecular weight of from about 900 to about 450,000 daltons, determined prior to substitution with the least one positively charged organic group. The poly alpha-1,6-glucan ether compound may be characterized by a degree of substitution of about 0.001 to about 3.0. Optionally, at least 3%, preferably from about 5% to about 50%, more preferably from about 5% to about 35%, of the backbone glucose monomer units have branches via alpha-1,2 and/or alpha-1,3-glycosidic linkages. These compounds, groups, and properties are described in more detail below.

The poly alpha-1,6-glucan ether compounds disclosed herein comprise poly alpha-1,6-glucan substituted with at least one positively charged organic group, wherein the organic group or groups are independently linked to the poly alpha-1,6-glucan polysaccharide backbone and/or to any branches, if present, through an ether (-O-) linkage. The at least one positively charged organic group can derivatize the poly alpha-1,6-glucan at the 2, 3, and/or 4 glucose carbon position(s) of a glucose monomer on the backbone of the glucan, and/or at the 1, 2, 3, 4, or 6 glucose carbon position(s) of a glucose monomer on a branch, if present. At unsubstituted positions a hydroxyl group is present in a glucose monomer.

The poly alpha-1,6-glucan ether compounds disclosed herein are referred to as "cationic" ether compounds due to the presence of one or more positively charged organic groups. The terms "positively charged organic group", "positively charged ionic group", and "cationic group" are used interchangeably herein. A positively charged group comprises a cation (a positively charged ion). Examples of positively charged groups include substituted ammonium groups, carbocation groups, and acyl cation groups.

The cationic poly alpha-1,6-glucan ether compounds disclosed herein comprise water-soluble poly alpha-1,6-glucan comprising a backbone of glucose monomer units wherein at least 65% of the glucose monomer units are linked via alpha-1,6-glycosidic linkages, and optionally at least 5% of the backbone glucose monomer units have branches via alpha-1,2 and/or alpha-1,3-glycosidic linkages. The poly alpha-1,6-glucan is substituted with positively charged organic groups on the polysaccharide backbone and/or on any branches which may be present, such that the poly alpha-1,6-glucan ether compound comprises unsubstituted and substituted alpha-D-glucose rings. The poly alpha-1,6-glucan may be randomly substituted with positively charged organic groups. As used herein, the term "randomly substituted" means the substituents on the glucose rings in the randomly substituted polysaccharide occur in a non-repeating or random fashion. That is, the substitution on a substituted glucose ring may be the same or different (i.e. the substituents, which may be the same or different, on different atoms in the glucose rings in the polysaccharide) from the substitution on a second substituted glucose ring in the polysaccharide, such that the overall substitution on the polymer has no pattern. Further, the substituted glucose rings may occur randomly within the polysaccharide (i.e., there is no pattern with the substituted and unsubstituted glucose rings within the polysaccharide).

Depending on reaction conditions and the specific substituent used to derivatize the poly alpha-1,6-glucan, the glucose monomers of the polymer backbone may be disproportionately substituted relative to the glucose monomers of any branches, including branches via alpha-1,2 and/or alpha-1,3 linkages, if present. The glucose monomers of the branches, including branches via alpha-1,2 and/or alpha-1,3 linkages, if present, may be disproportionately substituted relative to the glucose monomers of the polymer backbone. Depending on reaction conditions and the specific substituent used, substitution of the poly alpha-1,6-glucan may occur in a block manner.

Depending on reaction conditions and the specific substituent used to derivatize the poly alpha-1,6-glucan, it is possible that the hydroxyl groups at certain glucose carbon positions may be disproportionately substituted. For example, the hydroxyl at carbon position 6 for a branched unit may be more substituted than the hydroxyls at other carbon positions. The hydroxyl at carbon position 2, 3, or 4 may be more substituted than the hydroxyls at other carbon positions.

The poly alpha-1,6-glucan ether compounds disclosed herein contain positively charged organic groups and are of interest due to their solubility characteristics in water, which can be varied by appropriate selection of substituents and the degree of substitution. Compositions comprising the poly alpha-1,6-glucan ether compounds can be useful in a wide range of applications, including laundry, cleaning, food, cosmetics, industrial, film, and paper production. Poly alpha-1,6-glucan ether compounds having greater than 0.1 weight percent (wt %) solubility in water can be useful as rheology modifiers, emulsion stabilizers, and dispersing agents in cleaning, detergent, cosmetics, food, cement, film, and paper production, wherein the products are in a primarily water based formulation and optical clarity is desired. Poly alpha-1,6-glucan ether compounds having less than 0.1 wt% solubility in water can be useful as rheology modifiers, emulsion stabilizers, and dispersing agents in cleaning, detergent, cosmetics, food, cement, film, and paper production, wherein the products are in formulations which contain organic solvents to solubilize or disperse the poly alpha-1,6-glucan derivatives. The poly alpha-1,6-glucan ether compound may have a DoS of about 0.001 to about 1.5 and a solubility of 0.1% by weight or higher in deionized water at 25 °C. The poly alpha-1,6-glucan ether compound may have a DoS of about 0.05 to about 1.5 and a solubility of less than 0.1% by weight in pH 7 water at 25 °C. Poly alpha-1,6-glucan ether compounds having a solubility of at least 0.1%, or at least 1%, or at least 10%, or at least 25%, or at least 50%, or at least 75%, or at least 90%, by weight, in deionized water at 25 °C may be preferred for use in fabric care or dish care compositions, due to ease of processing and/or increased solubility in aqueous end-use conditions.

The cationic poly alpha-1,6-glucan ether compounds disclosed herein can be comprised in a water soluble unit dose fabric care composition in an effective amount, for example an amount that provides a desired degree of one or more of the following physical properties to the product or to the end-use: thickening, freeze/thaw stability, lubricity, moisture retention and release, texture, consistency, shape retention, emulsification, binding, suspension, dispersion, and/or gelation. Effective amounts may also be selected to provide treatment benefits in the desired end-use of the composition, for example deposition benefits, freshness benefits, softness or other conditioning benefits, color benefits, stain removal benefits, whiteness or anti-graying benefits.

The treatment composition comprises from 0.01% to 10%, preferably from 0.1% to 5%, or from 0.3% to 3%, or from 0.5% to 2.0%, by weight of the treatment composition, of the poly alpha-1,6-glucan ether compound.

The poly alpha-1,6-glucan ether compounds of the present disclosure comprise a substituted poly alpha-1,6-glucan, and are typically made from a poly alpha-1,6-glucan starting material. The terms "poly alpha-1,6-glucan" and "dextran" are used interchangeably herein. Dextrans represent a family of complex, branched alpha-glucans generally comprising chains of alpha-1,6-linked glucose monomers, with periodic side chains (branches) linked to the straight chains by alpha-1,3-linkage (Ioan et al., Macromolecules 33:5730-5739) or alpha-1,2-linkage. Production of dextrans is typically done through fermentation of sucrose with bacteria (e.g., *Leuconostoc* or *Streptococcus* species), where sucrose serves as the source of glucose for dextran polymerization (Naessens et al., J. Chem. Technol. Biotechnol. 80:845-860; Sarwat et al., Int. J. Biol. Sci. 4:379-386; Onilude et al., Int. Food Res. J. 20:1645-1651). Poly alpha-1,6-glucan can be prepared using glucosyltransferases such as (but not limited to) GTF1729, GTF1428, GTF5604, GTF6831, GTF8845, GTF0088, and GTF8117 as described in WO2015/183714 and WO2017/091533, both of which are incorporated herein by reference.

The cationic poly alpha-1,6-glucan ether compound may comprise a backbone of glucose monomer units wherein greater than or equal to 40% of the glucose monomer units are linked via alpha-1,6-glycosodic linkages, for example greater than or equal to 40%, 45%, 50%, 55%, 60%, 65%, 70%, 75%, 80%, 90%, or 95% of the glucose monomer units. The backbone of the cationic poly alpha-1,6-glucan ether compound can comprise at least 3%, 5%, 10%, 15%, 20%, 25%, 30%, 35%, 40%, 45%, 50%, 55%, or 60% glucose monomer units which are linked via alpha-1,2, alpha-1,3, and/or alpha-1,4 glycosidic linkages. The cationic poly alpha-1,6-glucan ether compound may comprise a backbone of glucose monomer units wherein at least 65% of the glucose monomer units are linked via alpha-1,6-glycosidic linkages. The cationic poly alpha-1,6-glucan ether compound may comprise a backbone of glucose monomer units wherein at least 70% of the glucose monomer units are linked via alpha-1,6-glycosidic linkages. The cationic poly alpha-1,6-glucan ether compound may comprise a backbone of glucose monomer units wherein at least 80% of the glucose monomer units are linked via alpha-1,6-glycosidic linkages. The cationic poly alpha-1,6-glucan ether compound may comprise a backbone of glucose monomer units wherein at least 90% of the glucose monomer units are linked via alpha-1,6-glycosidic linkages. The cationic poly alpha-1,6-glucan ether compound may comprise a backbone of glucose monomer units wherein at least 95% of the glucose monomer units are linked via alpha-1,6-glycosidic linkages. The cationic poly alpha-1,6-glucan ether compound may comprise a backbone of glucose monomer units wherein at least 99.5% of the glucose monomer units are linked via alpha-1,6-glycosidic linkages. The poly alpha-1,6-glucan ether compound may be predominantly linear.

Dextran "long chains" can comprise "substantially (or mostly) alpha-1,6-glucosidic linkages", meaning that they can have at least about 98.0% alpha-1,6-glucosidic linkages in some aspects. Dextran herein can comprise a "branching structure" (branched structure) in some aspects. It is contemplated that in this structure, long chains branch from other long chains, likely in an iterative manner (e.g., a long chain can be a branch from another long chain, which in turn can itself be a branch from another long chain, and so on). It is contemplated that long chains in this structure can be "similar in length", meaning that the length (e.g., measured by DP / degree of polymerization) of at least 70% of all the long chains in a branching structure is within plus/minus 30% of the mean length of all the long chains of the branching structure.

Dextran may further comprise "short chains" branching from the polysaccharide backbone, the branches typically being one to three glucose monomers in length, and typically comprising less than about 10% of all the glucose monomers of a dextran polymer. Such short chains typically comprise alpha-1,2-, alpha-1,3-, and/or alpha-1,4-glucosidic linkages (it is understood that there can also be a small percentage of such non-alpha-1,6 linkages in long chains in some aspects). The amount of alpha-1,2-branching or alpha-1,3-branching can be determined by NMR methods, as disclosed in the Test Methods.

Dextran can be produced enzymatically prior to being modified with alpha-1,2 or alpha-1,3 branches. In certain embodiments, dextran can be synthesized using a dextransucrase and/or methodology as disclosed in WO 2015/183714 or WO 2017/091533 or published application US 2018/0282385, which are all incorporated herein by reference. The dextransucrase identified as GTF8117, GTF6831, or GTF5604 in these references can be used, if desired (or any dextransucrase comprising an amino acid sequence that is at least about 90%, 91%, 92%, 93%, 94%, 95%, 96%, 97%, 98%, or 99% identical to any of these particular dextransucrases). Such enzymatically produced dextran is linear (i.e. 100% alpha-1,6-linkages) and aqueous soluble.

The poly-1,6-glucan with branching can be produced enzymatically according to the procedures in WO 2015/183714 and WO 2017/091533 where, for example, alpha-1,2-branching enzymes such as "gtfJ18T1" or "GTF9905" can be added during or after the production of the dextran polymer (polysaccharide). It may be that any other enzyme known to produce alpha-1,2-branching can be added. For example, poly-1,6-glucan with alpha-1,3-branching can be prepared as disclosed in Vuillemin et al. (2016, J. Biol Chem. 291:7687-7702) or U.S. Appl. No. 62/871,796, which are incorporated herein by reference. The degree of branching of poly alpha-1,6-glucan or its derivative has less than or equal to 50%, 40%, 30%, 20%, 10%, or 5% (or any value between 5% and 50%) of short branching, for example alpha-1,2- branching, 1,3-branching, or both alpha-1,2-branching and alpha-1,3-branching. The degree of branching in a poly alpha-1,6-glucan starting material is maintained in a branched poly alpha-1,6-glucan ether formed by etherification of the branched poly alpha-1,6-glucan. The amount of alpha-1,2-branching or alpha-1,3-branching can be determined by NMR methods, as disclosed in the Test Methods below.

Without wishing to be bound by theory, it is believed that branching can increase the solubility of the poly alph-1,6-glucan ether compound, which can lead to more convenient processability and/or transport. It is also believed that limits on the degree of branching can lead to improved performance in the final treatment composition.

A poly alpha-1,6-glucan ether compound may have a degree of alpha-1,2-branching that is less than 50%. A poly alpha-1,6-glucan ether compound may have a degree of alpha-1,2-branching that is at least 5%. From about 5% to about 50% of the backbone glucose monomer units of a poly alpha-1,6-glucan ether compound may have branches via alpha-1,2 or alpha-1,3 glycosidic linkages. From about 5% to about 35% of the backbone glucose monomer units of a poly alpha-1,6-glucan ether compound may have branches via alpha-1,2 or alpha-1,3 glycosidic linkages.

At least about 3%, preferably at least about 5% of the backbone glucose monomer units of a poly alpha-1,6-glucan ether compound may have branches via alpha-1,2- or alpha-1,3-glycosidic linkages. A poly alpha-1,6-glucan ether compound may comprise a backbone of glucose monomer units wherein greater than or equal to 65% of the glucose monomer units are linked via alpha-1,6-glycosidic linkages. A poly alpha-1,6-glucan ether compound may comprise a backbone of glucose monomer units wherein greater than or equal to 65% of the glucose monomer units are linked via alpha-1,6-glycosidic linkages and at least3%, preferably at least 5%, preferably from about 5% to about 30%, more preferably from about 5% to about 25%, even more preferably from about 5% to about 20%, of the glucose monomer units have branches via alpha-1,2- or alpha-1,3-glycosidic linkages. A poly alpha-1,6-glucan ether compound may comprise a backbone of glucose monomer units wherein greater than or equal to 65% of the glucose monomer units are linked via alpha-1,6-glycosidic linkages and at least 5% of the glucose monomer units have branches via alpha-1,2 linkages. A poly alpha-1,6-glucan ether compound may comprise a backbone of glucose monomer units wherein greater than or equal to 65% of the glucose monomer units are linked via alpha-1,6-glycosidic linkages and at least 5% of the glucose monomer units have branches via alpha-1,3 linkages. A poly alpha-1,6-glucan ether compound may comprise a backbone of glucose monomer units wherein greater than or equal to 65% of the glucose monomer units are linked via alpha-1,6-glycosidic linkages and from about 5% to about 50% of the glucose monomer units have branches via alpha-1,2- or alpha-1,3-glycosidic linkages. A poly alpha-1,6-glucan ether compound may comprise a backbone of glucose monomer units wherein greater than or equal to 70% of the glucose monomer units are linked via alpha-1,6-glycosidic linkages and from about 5% to about 35% of the glucose monomer units have branches via alpha-1,2- or alpha-1,3-glycosidic linkages.

A poly alpha-1,6-glucan ether compound may comprise a backbone of glucose monomer units wherein greater than or equal to 90% of the glucose monomer units are linked via alpha-1,6-glycosidic linkages. A poly alpha-1,6-glucan ether compound may comprise a backbone of glucose monomer units wherein greater than or equal to 90% of the glucose monomer units are linked via alpha-1,6-glycosidic linkages and at least 5% of the glucose monomer units have branches via alpha-1,2- or alpha-1,3-glycosidic linkages. A poly alpha-1,6-glucan ether compound may comprise a backbone of glucose monomer units wherein greater than or equal to 90% of the glucose monomer units are linked via alpha-1,6-glycosidic linkages and at least 5% of the glucose monomer units have branches via alpha-1,2 linkages. A poly alpha-1,6-glucan ether compound may comprise a backbone of glucose monomer units wherein greater than or equal to 90% of the glucose monomer units are linked via alpha-1,6-glycosidic linkages and at least 5% of the glucose monomer units have branches via alpha-1,3 linkages. A poly alpha-1,6-glucan ether compound may comprise a backbone of glucose monomer units wherein greater than or equal to 90% of the glucose monomer units are linked via alpha-1,6-glycosidic linkages and from about 5% to about 50% of the glucose monomer units have branches via alpha-1,2- or alpha-1,3-glycosidic linkages. A poly alpha-1,6-glucan ether compound may comprise a backbone of glucose monomer units wherein greater than or equal to 90% of the glucose monomer units are linked via alpha-1,6-glycosidic linkages and from about 5% to about 35% of the glucose monomer units have branches via alpha-1,2- or alpha-1,3-glycosidic linkages.

The poly alpha-1,6-glucan and poly alpha-1,6-glucan ether compounds disclosed herein can have a number average degree of polymerization (DPn) in the range of 5 to 6000. The DPn can be in the range of from 5 to 100, or from 5 to 500, or from 5 to 1000, or from 5 to 1500, or from 5 to 2000, or from 5 to 2500, or from 5 to 3000, or from 5 to 4000, or from 5 to 5000, or from 5 to 6000. The DPn can be in the range of from 50 to 500, or from 50 to 1000, or from 50 to 1500, or from 50 to 2000, or from 50 to 3000, or from 50 to 4000, or from 50 to 5000, or from 50 to 6000.

The poly alpha-1,6-glucan and poly alpha-1,6-glucan ether compounds disclosed herein can have a weight average degree of polymerization (DPw) in the range of at least 5. The DPw can be in the range of from 5 to 6000, or from 50 to 5000, or from 100 to 4000, or from 250 to 3000, or from 500 to 2000, or from 750 to 1500, or from 1000 to 1400, or from 1100 to 1300. The DPw can be in the range of from 400 to 6000, or from 400 to 5000, or from 400 to 4000, or from 400 to 3000, or from 400 to 2000, or from 400 to 1500.

The poly alpha-1,6-glucan ether compounds disclosed herein can have a weight average molecular weight of from about 1000 to about 500,000 daltons, or from about 10,000 to about 400,000 daltons, or from about 40,000 to about 300,000 daltons, or from about 80,000 to about 300,000 daltons, or from about 100,000 to about 250,000 daltons, or from about 150,000 to about 250,000 daltons, or from about 180,000 to about 225,000 daltons, or from about 180,000 to about 200,000 daltons. It may be that differently sized polymers may be preferred for different applications and/or intended benefits.

The poly alpha-1,6-glucan ether compounds disclosed herein can be derived from a poly alpha-1,6-glucan having a weight average molecular weight of from about 900 to about 450,000 daltons, determined prior to substitution with the least one positively charged organic group. The poly alpha-1,6-glucan ether compounds disclosed herein can be derived from a poly alpha-1,6-glucan having a weight average molecular weight of from about 5000 to about 400,000 daltons, or from about 10,000 to about 350,000 daltons, or from about 50,000 to about 350,000 daltons, or from about 90,000 to about 300,000 daltons, or from about 125,000 to about 250,000 daltons, or from about 150,000 to about 200,000 daltons. Differently sized feedstock or backbone polymers may be preferred for different applications, or depending on the intended degree of substitution.

The term "degree of substitution" (DoS) as used herein refers to the average number of hydroxyl groups substituted in each monomeric unit (glucose) of a cationic poly alpha-1,6-glucan ether compound, which includes the monomeric units within the backbone and within any alpha-1,2 or alpha-1,3 branches which may be present. Since there are at most three hydroxyl groups in a glucose monomeric unit in a poly alpha-1,6-glucan polymer or cationic poly alpha-1,6-glucan ether compound, the overall degree of substitution can be no higher than 3. It would be understood by those skilled in the art that, since a cationic poly alpha-1,6-glucan ether compound as disclosed herein can have a degree of substitution between about 0.001 to about 3.0, the substituents on the polysaccharide cannot only be hydroxyl. The degree of substitution of a poly alpha-1,6-glucan ether compound can be stated with reference to a specific substituent or with reference to the overall degree of substitution, that is, the sum of the DoS of each different substituent for an ether compound as defined herein. As used herein, when the degree of substitution is not stated with reference to a specific substituent or substituent type, the overall degree of substitution of the cationic poly alpha-1,6-glucan ether compound is meant. The degree of substitution may be a cationic degree of substitution, or even a net cationic degree of substitution. The target DoS can be chosen to provide the desired solubility and performance of a composition comprising a cationic poly alpha-1,6-glucan ether compound in the specific application of interest.

Cationic poly alpha-1,6-glucan ether compounds disclosed herein may have a DoS with respect to a positively charged organic group in the range of about 0.001 to about 3. A cationic poly alpha-1,6-glucan ether may have a DoS of about 0.01 to about 1.5. The poly alpha-1,6-glucan ether may have a DoS of about 0.01 to about 0.7. The poly alpha-1,6-glucan ether may have a DoS of about 0.01 to about 0.4. The poly alpha-1,6-glucan ether may have a DoS of about 0.01 to about 0.2. The DoS of the poly alpha-1,6-glucan ether compound can be at least about 0.001, 0.005, 0.1, 0.15, 0.2, 0.3, 0.4, 0.5, 0.6, 0.7, 0.8, 0.9, 1.0, 1.1, 1.2, 1.3, 1.4, 1.5, 1.6, 1.7, 1.8, 1.9, 2.0, 2.1, 2.2, 2.3, 2.4, 2.5, 2.6, 2.7, 2.8, 2.9, or 3.0. The DoS may be from about 0.01 to about 1.5, preferably from about 0.01 to about 1.0, more preferably from about 0.01 to about 0.8, more preferably from about 0.03 to about 0.7, or from about 0.04 to about 0.6, or from about 0.05 to about 0.5. For performance reasons in through-the-wash applications (e.g., a laundry detergent used in a wash cycle), it may be preferable for the DoS to be from about 0.01 to about 0.5, or from about 0.01 to about 0.25, or from about 0.01 to about 0.2, or from about 0.03 to about 0.15, or from about 0.04 to about 0.12. For performance reasons in through-the-rinse applications (e.g., a liquid fabric enhancer used in a rinse cycle), it may be preferably for the DoS to be from about 0.01 to about 1, or from about 0.03 to about 0.8, or from about 0.04 to about 0.7, or from about 0.05 to about 0.6, or from about 0.2 to about 0.8, or from about 0.2 to about 0.6, or from about 0.3 to about 0.6, or from about 0.4 to about 0.6. The DoS of the poly alpha-1,6-glucan may be from 0.01 to about 0.6, more preferably from 0.02 to about 0.5.

The cationic poly alpha-1,6-glucan ether compounds of the present disclosure may be characterized by a cationic charge density. Cationic charge density may be expressed as milliequivalents of charge per gram of compound (meq/mol) and may be determined according to the method provided in the Test Methods section. The cationic poly alpha-1,6-glucan ether compounds of the present disclosure may be characterized by a cationic charge density (or "CCD") of from about 0.05 to about 12 meq/g, or from about 0.1 to about 8 meq/g, or from about 0.1 to about 4 meq/g, or from about 0.1 to about 3 meq/g, or from about 0.1 to about 2.6 meq/g.

A positively charged organic group comprises a chain of one or more carbons having one or more hydrogens substituted with another atom or functional group, wherein one or more of the substitutions is with a positively charged group. The term "chain" as used herein encompasses linear, branched, and cyclic arrangements of carbon atoms, as well as combinations thereof.

The poly alpha-1,6-glucan derivative comprises poly alpha-1,6-glucan substituted with at least one positively charged organic group on the polysaccharide backbone and/or on one or more of the optional branches. When substitution occurs on a glucose monomer contained in the backbone, the polysaccharide is derivatized at the 2, 3, and/or 4 glucose carbon position(s) with an organic group as defined herein which is linked to the polysaccharide through an ether (-O-) linkage in place of the hydroxyl group originally present in the underivatized (unsubstituted) poly alpha-1,6-glucan. When substitution occurs on a glucose monomer contained in a branch, the polysaccharide is derivatized at the 1, 2, 3, 4, or 6 glucose carbon position(s) with a positively charged organic group as defined herein which is linked to the polysaccharide through an ether (-O-) linkage.

A poly alpha-1,6-glucan ether compound as disclosed herein is termed a glucan "ether" herein by virtue of comprising the substructure -C_{G}-O-C_{R}-, wherein "-C_{G}-" represents a carbon of a glucose monomer unit of a poly alpha-1,6-glucan ether compound, and wherein "-C_{R}-" is comprised in the positively charged organic group. A cationic poly alpha-1,6-glucan monoether contains one type of a positively charged organic group. A cationic poly alpha-1,6-glucan mixed ether contains two or more types of positively charged organic groups. Mixtures of cationic poly alpha-1,6-glucan ether compounds can also be used.

Treatment compositions disclosed herein can comprise, or consist essentially of, one or more cationic poly alpha-1,6-glucan ether compounds as disclosed herein. A treatment composition may comprise one poly alpha-1,6-glucan ether compound. A treatment composition may comprise two or more poly alpha-1,6-glucan ether compounds, for example wherein the positively charged organic groups are different.

A treatment composition may comprise one or more cationic poly alpha-1,6-glucan ether compounds as disclosed herein, and may further comprise unsubstituted and/or non-cationic poly alpha-1,6-glucan compounds, which may be residual reactants that are unreacted/unsubstituted, or may have hydrolyzed. Typically, a low level of unsubstituted/non-cationic poly alpha-1,6-glucan compounds is preferred, as low levels may be indicative of reaction completeness with regard to the substitution, and/or chemical stability of the compounds in the treatment composition. The weight ratio of the cationic poly alpha-1,6-glucan ether compounds to unsubstituted/non-cationic poly alpha 1,6-glucan compounds may be 95:5 or greater, preferably 98:2 or greater, more preferably 99:1 or greater.

A "positively charged organic group" as used herein refers to a chain of one or more carbons that has one or more hydrogens substituted with another atom or functional group, wherein one or more of the substitutions is with a positively charged group. A positively charged group is typically bonded to the terminal carbon atom of the carbon chain. A positively charged organic group is considered to have a net positive charge since it comprises one or more positively charged groups, and comprises a cation (a positively charged ion). An organic group or compound that is "positively charged" typically has more protons than electrons and is repelled from other positively charged substances, but attracted to negatively charged substances. An example of a positively charged groups includes a substituted ammonium group. A positively charged organic group may have a further substitution, for example with one or more hydroxyl groups, oxygen atoms (forming a ketone group), alkyl groups, and/or at least one additional positively charged group.

A positively charged organic group may comprise a substituted ammonium group, which can be represented by Structure II:

In Structure II, R₂, R₃ and R₄ may each independently represent a hydrogen atom, an alkyl group, or a C₆-C₂₄ aryl group. The carbon atom (C) shown in Structure II is part of the carbon chain of the positively charged organic group. The carbon atom is either directly ether-linked to a glucose monomer of poly alpha-1,6-glucan, or is part of a chain of two or more carbon atoms ether-linked to a glucose monomer of poly alpha-1,6-glucan. The carbon atom shown in Structure II can be -CH₂-, -CH- (where a H is substituted with another group such as a hydroxy group), or -C- (where both H's are substituted).

When R₂, R₃ and/or R₄ represent an alkyl group, the alkyl group can be a C₁-C₃₀ alkyl group, for example a methyl, ethyl, propyl, butyl, pentyl, hexyl, heptyl, octyl, nonyl, decyl, undecyl, dodecyl, tridecyl, tetradecyl, pentadecyl, hexadecyl, heptadecyl, octadecyl, nonadecyl, icosyl, henicosyl, docosyl, tricosyl, tetracosyl, C₂₅, C₂₆, C₂₇, C₂₈, C₂₉, or C₃₀ group. The alkyl group can be a C₁-C₂₄ alkyl group, or a C₁-C₁₈ or a C₆-C₂₀ alkyl group, or a C₁₀-C₁₆ alkyl group, or a C₁-C₄ alkyl group. When a positively charged organic group comprises a substituted ammonium group which has two or more alkyl groups, each alkyl group can be the same as or different from the other.

When R₂, R₃ and/or R₄ represent an aryl group, the aryl group can be a C₆-C₂₄ aryl group, optionally substituted with alkyl substituents. The aryl group can be a C₁₂-C₂₄ aryl group, optionally substituted with alkyl substituents, or a C₆-C₁₈ aryl group, optionally substituted with alkyl substituents.

A substituted ammonium group can be a "primary ammonium group", "secondary ammonium group", "tertiary ammonium group", or "quaternary ammonium" group, depending on the composition of R₂, R₃ and R₄ in Structure II. A primary ammonium group is an ammonium group represented by Structure II in which each of R₂, R₃ and R₄ is a hydrogen atom (i.e., -C-NH₃⁺).

A secondary ammonium group is an ammonium group represented by Structure II in which each of R₂ and R₃ is a hydrogen atom and R₄ is a C₁-C₃₀ alkyl group or a C₆-C₂₄ aryl group. A "secondary ammonium poly alpha-1,6-glucan ether compound" comprises a positively charged organic group having a monoalkylammonium group. A secondary ammonium poly alpha-1,6-glucan ether compound can be represented in shorthand as a monoalkylammonium poly alpha-1,6-glucan ether, for example monomethyl-, monoethyl-, monopropyl-, monobutyl-, monopentyl-, monohexyl-, monoheptyl-, monooctyl-, monononyl-, monodecyl-, monoundecyl-, monododecyl-, monotridecyl-, monotetradecyl-, monopentadecyl-, monohexadecyl-, monoheptadecyl-, or monooctadecyl- ammonium poly alpha-1,6-glucan ether. These poly alpha-1,6-glucan ether compounds can also be referred to as methyl-, ethyl-, propyl-, butyl-, pentyl-, hexyl-, heptyl-, octyl-, nonyl-, decyl-, undecyl-, dodecyl-, tridecyl-, tetradecyl-, pentadecyl-, hexadecyl-, heptadecyl-, or octadecyl- ammonium poly alpha-1,6-glucan ether compounds, respectively. An octadecyl ammonium group is an example of a monoalkylammonium group wherein each of R₂ and R₃ is a hydrogen atom and R₄ is an octadecyl group. It would be understood that a second member (i.e., R₁) implied by "secondary" in the above nomenclature is the chain of one or more carbons of the positively charged organic group that is ether-linked to a glucose monomer of poly alpha-1,6-glucan.

A tertiary ammonium group is an ammonium group represented by Structure II in which R₂ is a hydrogen atom and each of R₃ and R₄ is independently a C₁-C₂₄ alkyl group or a C₆-C₂₄ aryl group. The alkyl groups can be the same or different. A "tertiary ammonium poly alpha-1,6-glucan ether compound" comprises a positively charged organic group having a dialkylammonium group. A tertiary ammonium poly alpha-1,6-glucan ether compound can be represented in shorthand as a dialkylammonium poly alpha-1,6-glucan ether, for example dimethyl-, diethyl-, dipropyl-, dibutyl-, dipentyl-, dihexyl-, diheptyl-, dioctyl-, dinonyl-, didecyl-, diundecyl-, didodecyl-, ditridecyl-, ditetradecyl-, dipentadecyl-, dihexadecyl-, diheptadecyl-, or dioctadecyl- ammonium poly alpha-1,6-glucan ether. A didodecyl ammonium group is an example of a dialkyl ammonium group, wherein R₂ is a hydrogen atom and each of R₃ and R₄ is a dodecyl group. It would be understood that a third member (i.e., R₁) implied by "tertiary" in the above nomenclature is the chain of one or more carbons of the positively charged organic group that is ether-linked to a glucose monomer of poly alpha-1,6-glucan.

A quaternary ammonium group is an ammonium group represented by Structure II in which each of R₂, R₃ and R₄ is independently a C₁-C₃₀ alkyl group or a C₆-C₂₄ aryl group (i.e., none of R₂, R₃ and R₄ is a hydrogen atom).

A quaternary ammonium poly alpha-1,6-glucan ether compound may comprise a trialkyl ammonium group, where each of R₂, R₃ and R₄ is independently a C₁-C₃₀ alkyl group. The alkyl groups can all be the same, or two of the alkyl groups can be the same and one different from the others, or all three alkyl groups can be different from one another. A quaternary ammonium poly alpha-1,6-glucan ether compound can be represented in shorthand as a trialkylammonium poly alpha-1,6-glucan ether, for example trimethyl-, triethyl-, tripropyl-, tributyl-, tripentyl-, trihexyl-, triheptyl-, trioctyl-, trinonyl-, tridecyl-, triundecyl-, tridodecyl-, tritridecyl-, tritetradecyl-, tripentadecyl-, trihexadecyl-, triheptadecyl-, or trioctadecyl- ammonium poly alpha-1,6-glucan ether. It would be understood that a fourth member (i.e., R₁) implied by "quaternary" in this nomenclature is the chain of one or more carbons of the positively charged organic group that is ether-linked to a glucose monomer of poly alpha-1,6-glucan. A trimethylammonium group is an example of a trialkyl ammonium group, wherein each of R₂, R₃ and R₄ is a methyl group.

A positively charged organic group comprising a substituted ammonium group represented by Structure II can have each of R₂, R₃ and R₄ independently represent a hydrogen atom or an aryl group, such as a phenyl or naphthyl group, or an aralkyl group such as a benzyl group, or a cycloalkyl group such as cyclohexyl or cyclopentyl. Each of R₂, R₃ and R₄ may further comprise an amino group or a hydroxyl group.

The substituted ammonium group of the positively charged organic group is a substituent on a chain of one or more carbons that is ether-linked to a glucose monomer of the alpha-1,6-glucan. The carbon chain may contain from one to 30 carbon atoms. The carbon chain may be linear. Examples of linear carbon chains include, for example, -CH₂-, -CH₂CH₂-, -CH₂CH₂CH₂-, -CH₂(CH₂)₂CH₂-, -CH₂(CH₂)₃CH₂-, -CH₂(CH₂)₄CH₂-, -CH₂(CH₂)₅CH₂-, -CH₂(CH₂)₆CH₂-, -CH₂(CH₂)₇CH₂-, -CH₂(CH₂)₈CH₂-, -CH₂(CH₂)₉CH₂-, and -CH₂(CH₂)₁₀CH₂-; longer carbon chains can also be used, if desired. The carbon chain may be branched, meaning the carbon chain is substituted with one or more alkyl groups, for example methyl, ethyl, propyl, or butyl groups. The point of substitution can be anywhere along the carbon chain. Examples of branched carbon chains include -CH(CH₃)CH₂-, -CH(CH₃)CH₂CH₂-, -CH₂CH(CH₃)CH₂-, - CH(CH₂CH₃)CH₂-, -CH(CH₂CH₃)CH₂CH₂-, -CH₂CH(CH₂CH₃)CH₂-, -CH(CH₂CH₂CH₃)CH₂-, -CH(CH₂CH₂CH₃)CH₂CH₂-, and -CH₂CH(CH₂CH₂CH₃)CH₂-; longer branched carbon chains can also be used, if desired. Where the positively charged group is a substituted ammonium group, the first carbon atom in the chain is ether-linked to a glucose monomer of the poly alpha-1,6-glucan, and the last carbon atom of the chain in each of these examples is represented by the C in Structure II.

The chain of one or more carbons may be further substituted with one or more hydroxyl groups. Examples of a carbon chain having one or more substitutions with a hydroxyl group include hydroxyalkyl (e.g., hydroxyethyl, hydroxypropyl, hydroxybutyl, hydroxypentyl, hydroxyhexyl, hydroxyheptyl, hydroxyoctyl) groups and dihydroxyalkyl (e.g., dihydroxyethyl, dihydroxypropyl, dihydroxybutyl, dihydroxypentyl, dihydroxyhexyl, dihydroxyheptyl, dihydroxyoctyl) groups. Examples of hydroxyalkyl and dihydroxyalkyl (diol) carbon chains include -CH(OH)-, -CH(OH)CH₂-, -C(OH)₂CH₂-, -CH₂CH(OH)CH₂-, -CH(OH)CH₂CH₂-, -CH(OH)CH(OH)CH₂-, -CH₂CH₂CH(OH)CH₂-, -CH₂CH(OH)CH₂CH₂-, -CH(OH)CH₂CH₂CH₂-, -CH₂CH(OH)CH(OH)CH₂-, -CH(OH)CH(OH)CH₂CH₂- and -CH(OH)CH₂CH(OH)CH₂-. In each of these examples, the first carbon atom of the chain is ether-linked to a glucose monomer of poly alpha-1,6-glucan, and the last carbon atom of the chain is linked to a positively charged group. Where the positively charged group is a substituted ammonium group, the last carbon atom of the chain in each of these examples is represented by the C in Structure II.

An example of a quaternary ammonium poly alpha-1,6-glucan ether compound is trimethylammonium hydroxypropyl poly alpha-1,6-glucan. The positively charged organic group of this ether compound can be represented by the following structure: where each of R₂, R₃ and R₄ is a methyl group. The structure above is an example of a quaternary ammonium hydroxypropyl group.

Where a carbon chain of a positively charged organic group has a substitution in addition to a substitution with a positively charged group, such additional substitution may be with one or more hydroxyl groups, oxygen atoms (thereby forming an aldehyde or ketone group), alkyl groups (e.g., methyl, ethyl, propyl, butyl), and/or additional positively charged groups. A positively charged group is typically bonded to the terminal carbon atom of the carbon chain. A positively charged group can also comprise one or more imidazoline rings.

A cationic poly alpha-1,6-glucan ether compound as disclosed herein may be a salt. The counter ion for the positively charged organic group can be any suitable anion, including an acetate, borate, bromate, bromide, carbonate, chlorate, chloride, chlorite, dihydrogen phosphate, fluoride, hydrogen carbonate, hydrogen phosphate, hydrogen sulfate, hydrogen sulfide, hydrogen sulfite, hydroxide, hypochlorite, iodate, iodide, nitrate, nitride, nitrite, oxalate, oxide, perchlorate, permanganate, phosphate, phosphide, phosphite, silicate, stannate, stannite, sulfate, sulfide, sulfite, tartrate, or thiocyanate anion, preferably chloride. In an aqueous solution, a poly alpha-1,6-glucan ether compound is in a cationic form. The positively charged organic groups of a cationic poly alpha-1,6-glucan ether compound can interact with salt anions that may be present in an aqueous solution.

The poly alpha-1,6-glucan ether compound may comprise a positively charged organic group, wherein the positively charged organic group comprises a substituted ammonium group. From about 0.5% to about 50% of the backbone glucose monomer units of the ether compound may have branches via alpha-1,2 glycosidic linkages, and the positively charged organic group may comprise a substituted ammonium group. From about 5% to about 30% of the backbone glucose monomer units of the ether compound may have branches via alpha-1,2 glycosidic linkages, and the substituted ammonium group may comprise a substituted ammonium group. From about 0.5% to about 50% of the backbone glucose monomer units of the ether compound may have branches via alpha-1,2 glycosidic linkages, and the substituted ammonium group may comprise a trimethyl ammonium group. From about 5% to about 35% of the backbone glucose monomer units of the ether compound may have branches via alpha-1,2 glycosidic linkages, and the substituted ammonium group may comprise a trimethyl ammonium group.

The poly alpha-1,6-glucan ether compound may comprise a positively charged organic group, wherein the positively charged organic group comprises a trimethylammonium hydroxyalkyl group. From about 0.5% to about 50% of the backbone glucose monomer units of the ether compound may have branches via alpha-1,2 glycosidic linkages, and the positively charged organic group may comprise a trimethylammonium hydroxyalkyl group. From about 5% to about 30% of the backbone glucose monomer units of the ether compound may have branches via alpha-1,2 glycosidic linkages, and the positively charged organic group may comprise a trimethylammonium hydroxyalkyl group. From about 0.5% to about 50% of the backbone glucose monomer units of the ether compound may have branches via alpha-1,2 glycosidic linkages, and the trimethylammonium hydroxyalkyl group may comprise a trimethylammonium hydroxypropyl group. From about 5% to about 30% of the backbone glucose monomer units of the ether compound may have branches via alpha-1,2 glycosidic linkages, and the trimethylammonium hydroxyalkyl group may comprise a trimethylammonium hydroxypropyl group.

The poly alpha-1,6-glucan ether compound may comprise a positively charged organic group, wherein the positively charged organic group comprises a substituted ammonium group comprising a quaternary ammonium group. From about 0.5% to about 50% of the backbone glucose monomer units of the ether compound may have branches via alpha-1,2 glycosidic linkages, and the quaternary ammonium group may comprise at least one C₁ to C₁₈ alkyl group. From about 5% to about 30% of the backbone glucose monomer units of the ether compound may have branches via alpha-1,2 glycosidic linkages, the quaternary ammonium group may comprise at least one C₁ to C₁₈ alkyl group. From about 0.5% to about 50% of the backbone glucose monomer units of the ether compound may have branches via alpha-1,2 glycosidic linkages, and the quaternary ammonium group may comprise at least one C₁ to C₄ alkyl group. From about 5% to about 30% of the backbone glucose monomer units of the ether compound may have branches via alpha-1,2 glycosidic linkages, and the quaternary ammonium group may comprise at least one C₁ to C₄ alkyl group. From about 0.5% to about 50% of the backbone glucose monomer units of the ether compound may have branches via alpha-1,2 glycosidic linkages, and the quaternary ammonium group may comprise at least one C₁₀ to C₁₆ alkyl group. From about 5% to about 30% of the backbone glucose monomer units of the ether compound may have branches via alpha-1,2 glycosidic linkages, and the quaternary ammonium group may comprise at least one C₁₀ to C₁₆ alkyl group.

The poly alpha-1,6-glucan ether compound may comprise a quaternary ammonium group comprising one C₁₀ to C₁₆ alkyl group, where the quaternary ammonium group further comprises two methyl groups. From about 0.5% to about 50% of the backbone glucose monomer units of the ether compound may have branches via alpha-1,2 glycosidic linkages, and the quaternary ammonium group may comprise one C₁₀ to C₁₆ alkyl group further comprises two methyl groups. From about 5% to about 30% of the backbone glucose monomer units of the ether compound may have branches via alpha-1,2 glycosidic linkages, and the quaternary ammonium group may comprise one C₁₀ to C₁₆ alkyl group further comprises two methyl groups.

From about 0.5% to about 50% of the backbone glucose monomer units of the ether compound may have branches via alpha-1,2 glycosidic linkages, and the quaternary ammonium group may comprise one C₁₀ alkyl group and two methyl groups. From about 5% to about 30% of the backbone glucose monomer units of the ether compound may have branches via alpha-1,2 glycosidic linkages, and the quaternary ammonium group may comprise one C₁₀ alkyl group and two methyl groups.

The poly alpha-1,6-glucan ether compound may comprise a positively charged organic group, wherein the positively charged organic group comprises a quaternary ammonium hydroxyalkyl group. From about 0.5% to about 50% of the backbone glucose monomer units of the ether compound may have branches via alpha-1,2 glycosidic linkages, and the positively charged organic group may comprise a quaternary ammonium hydroxyalkyl group. From about 5% to about 30% of the backbone glucose monomer units of the ether compound may have branches via alpha-1,2 glycosidic linkages, and the positively charged organic group may comprise a quaternary ammonium hydroxyalkyl group. From about 0.5% to about 50% of the backbone glucose monomer units of the ether compound may have branches via alpha-1,2 glycosidic linkages, and the quaternary ammonium hydroxyalkyl group may comprise a quaternary ammonium hydroxymethyl group, a quaternary ammonium hydroxyethyl group, or a quaternary ammonium hydroxypropyl group. From about 5% to about 30% of the backbone glucose monomer units of the ether compound may have branches via alpha-1,2 glycosidic linkages, and the quaternary ammonium hydroxyalkyl group may comprise a quaternary ammonium hydroxymethyl group, a quaternary ammonium hydroxyethyl group, or a quaternary ammonium hydroxypropyl group. From about 0.5% to about 50% of the backbone glucose monomer units of the ether compound may have branches via alpha-1,2 glycosidic linkages, and the quaternary ammonium hydroxyalkyl group may comprise a quaternary ammonium hydroxymethyl group. From about 5% to about 30% of the backbone glucose monomer units of the ether compound may have branches via alpha-1,2 glycosidic linkages, and the quaternary ammonium hydroxyalkyl group may comprise a quaternary ammonium hydroxymethyl group. From about 0.5% to about 50% of the backbone glucose monomer units of the ether compound may have branches via alpha-1,2 glycosidic linkages, and the quaternary ammonium hydroxyalkyl group may comprise a quaternary ammonium hydroxyethyl group. From about 5% to about 30% of the backbone glucose monomer units of the ether compound may have branches via alpha-1,2 glycosidic linkages, and the quaternary ammonium hydroxyalkyl group may comprise a quaternary ammonium hydroxyethyl group. From about 0.5% to about 50% of the backbone glucose monomer units of the ether compound may have branches via alpha-1,2 glycosidic linkages, and the quaternary ammonium hydroxyalkyl group may comprise a quaternary ammonium hydroxypropyl group. From about 5% to about 30% of the backbone glucose monomer units of the ether compound may have branches via alpha-1,2 glycosidic linkages, and the quaternary ammonium hydroxyalkyl group may comprise a quaternary ammonium hydroxypropyl group.

Poly alpha-1,6-glucan ether compounds containing a positively charged organic group, such as a trimethyl ammonium group, a substituted ammonium group, or a quaternary ammonium group, can be prepared using methods similar to those disclosed in published patent application US 2016/0311935, which is incorporated herein by reference in its entirety. US 2016/0311935 discloses poly alpha-1,3-glucan ether compounds comprising positively charged organic groups and having a degree of substitution of up to about 3.0, as well as methods of producing such ether compounds. Cationic poly alpha-1,6-glucan ethers may be prepared by contacting poly alpha-1,6-glucan with at least one etherification agent comprising a positively charged organic group under alkaline conditions. For example, alkaline conditions may be prepared by contacting the poly alpha-1,6-glucan with a solvent and one or more alkali hydroxides to provide a solution or mixture, and at least one etherification agent is then added. As another example, at least one etherification agent can be contacted with poly alpha-1,6-glucan and solvent, and then the alkali hydroxide can be added. The mixture of poly alpha-1,6-glucan, etherification agent, and alkali hydroxides can be maintained at ambient temperature or optionally heated, for example to a temperature between about 25 °C and about 200 °C, depending on the etherification agent and/or solvent employed. Reaction time for producing a poly alpha-1,6-glucan ether will vary corresponding to the reaction temperature, with longer reaction time necessary at lower temperatures and lower reaction time necessary at higher temperatures.

Typically, the solvent comprises water. Optionally, additional solvent can be added to the alkaline solution, for example alcohols such as isopropanol, acetone, dioxane, and toluene. Alternatively, solvents such as lithium chloride(LiCl)/N,N-dimethyl-acetamide (DMAc), SO₂/diethylamine (DEA)/dimethyl sulfoxide (DMSO), LiCl/1,3-dimethy-2-imidazolidinone (DMI), N,N-dimethylformamide (DMF)/N₂O₄, DMSO/tetrabutyl-ammonium fluoride trihydrate (TBAF), N-methylmorpholine-N-oxide (NMMO), Ni(tren)(OH)₂ [tren-tris(2-aminoethyl)amine] aqueous solutions and melts of LiClO₄·3H₂O, NaOH/urea aqueous solutions, aqueous sodium hydroxide, aqueous potassium hydroxide, formic acid, and ionic liquids can be used.

An etherification agent may be one that can etherify poly alpha-1,6-glucan with a positively charged organic group, where the carbon chain of the positively charged organic group only has a substitution with a positively charged group (e.g., substituted ammonium group such as trimethylammonium). Examples of such etherification agents include dialkyl sulfates, dialkyl carbonates, alkyl halides (e.g., alkyl chloride), iodoalkanes, alkyl triflates (alkyl trifluoromethanesulfonates) and alkyl fluorosulfonates, where the alkyl group(s) of each of these agents has one or more substitutions with a positively charged group (e.g., substituted ammonium group such as trimethylammonium). Other examples of such etherification agents include dimethyl sulfate, dimethyl carbonate, methyl chloride, iodomethane, methyl triflate and methyl fluorosulfonate, where the methyl group(s) of each of these agents has a substitution with a positively charged group (e.g., substituted ammonium group such as trimethylammonium). Other examples of such etherification agents include diethyl sulfate, diethyl carbonate, ethyl chloride, iodoethane, ethyl triflate and ethyl fluorosulfonate, where the ethyl group(s) of each of these agents has a substitution with a positively charged group (e.g., substituted ammonium group such as trimethylammonium). Other examples of such etherification agents include dipropyl sulfate, dipropyl carbonate, propyl chloride, iodopropane, propyl triflate and propyl fluorosulfonate, where the propyl group(s) of each of these agents has one or more substitutions with a positively charged group (e.g., substituted ammonium group such as trimethylammonium). Other examples of such etherification agents include dibutyl sulfate, dibutyl carbonate, butyl chloride, iodobutane and butyl triflate, where the butyl group(s) of each of these agents has one or more substitutions with a positively charged group (e.g., substituted ammonium group such as trimethylammonium). Other examples of etherification agents include halides of imidazoline-ring-containing compounds.

An etherification agent may be one that can etherify poly alpha-1,6-glucan with a positively charged organic group, where the carbon chain of the positively charged organic group has a substitution, for example a hydroxyl group, in addition to a substitution with a positively charged group, for example a substituted ammonium group such as trimethylammonium. Examples of such etherification agents include hydroxyalkyl halides (e.g., hydroxyalkyl chloride) such as hydroxypropyl halide and hydroxybutyl halide, where a terminal carbon of each of these agents has a substitution with a positively charged group (e.g., substituted ammonium group such as trimethylammonium); an example is 3-chloro-2-hydroxypropyltrimethylammonium. Additional examples of etherification agents comprising a positively charged organic group include 2,3-epoxypropyltrimethylammonium chloride, 3-chloro-2-hydroxypropyl dodecyldimethylammonium chloride, 3-chloro-2-hydroxypropyl cocoalkyldimethylammonium chloride, 3-chloro-2-hydroxypropyl stearyldimethylammonium chloride, and quaternary ammonium compounds such as halides of imidazoline-ring-containing compounds. Other examples of such etherification agents include alkylene oxides such as propylene oxide (e.g., 1,2-propylene oxide) and butylene oxide (e.g., 1,2-butylene oxide; 2,3-butylene oxide), where a terminal carbon of each of these agents has a substitution with a positively charged group (e.g., substituted ammonium group such as trimethylammonium).

When producing a poly alpha-1,6-glucan ether compound comprising two or more different positively charged organic groups, two or more different etherification agents would be used, accordingly. Any of the etherification agents disclosed herein may be combined to produce poly alpha-1,6-glucan ether compounds having two or more different positively charged organic groups. Such two or more etherification agents may be used in the reaction at the same time, or may be used sequentially in the reaction. When used sequentially, any of the temperature-treatment (e.g., heating) steps may optionally be used between each addition. Sequential introduction of etherification agents may be used to control the desired DoS of each positively charged organic group. In general, a particular etherification agent would be used first if the organic group it forms in the ether product is desired at a higher DoS compared to the DoS of another organic group to be added.

The amount of etherification agent to be contacted with poly alpha-1,6-glucan in a reaction under alkaline conditions can be selected based on the degree of substitution desired in the ether compound. The amount of ether substitution groups on each monomeric unit in poly alpha-1,6-glucan ether compounds can be determined using nuclear magnetic resonance (NMR) spectroscopy. In general, an etherification agent can be used in a quantity of at least about 0.05 mole per mole of poly glucan. There may be no upper limit to the quantity of etherification agent that can be used.

Reactions for producing poly alpha-1,6-glucan ether compounds can optionally be carried out in a pressure vessel such as a Parr reactor, an autoclave, a shaker tube, or any other pressure vessel well known in the art. Optionally, poly alpha-1,6-glucan ether compounds can be prepared under an inert atmosphere, with or without heating. As used herein, the term "inert atmosphere" refers to a nonreactive gas atmosphere such as nitrogen, argon, or helium.

After contacting the poly alpha-1,6-glucan, solvent, alkali hydroxide, and etherification reagent for a sufficient reaction time to produce a poly alpha-1,6-glucan ether compound, the reaction mixture can optionally be filtered by any means known in the art which allows removal of liquids from solids.

Following etherification, one or more acids may be optionally added to the reaction mixture to lower the pH to a neutral pH range that is neither substantially acidic nor substantially acidic, for example a pH of about 6-8, or about 6.0, 6.2, 6.4, 6.6, 6.8, 7.0, 7.2, 7.4, 7.6, 7.8, or 8.0, if desired. Various acids useful for this purpose include sulfuric, acetic, hydrochloric, nitric, any mineral (inorganic) acid, any organic acid, or any combination of these acids.

A poly alpha-1,6-glucan ether compound can optionally be washed one or more times with a liquid that does not readily dissolve the compound. For example, a poly alpha-1,6-glucan ether can be washed with water, alcohol, isopropanol, acetone, aromatics, or any combination of these, depending on the solubility of the ether compound therein (where lack of solubility is desirable for washing). In general, a solvent comprising an organic solvent such as alcohol is preferred for the washing. A poly alpha-1,6-glucan ether product can be washed one or more times with an aqueous solution containing methanol or ethanol, for example. For example, 70-95 wt% ethanol can be used to wash the product. In another embodiment, a poly alpha-1,6-glucan ether product can be washed with a methanol: acetone (e.g., 60:40) solution.

A poly alpha-1,6-glucan ether compound can optionally purified by membrane filtration.

A poly alpha-1,6-glucan ether produced using the methods disclosed above can be isolated. This step can be performed before or after neutralization and/or washing steps using a funnel, centrifuge, press filter, or any other method or equipment known in the art that allows removal of liquids from solids. An isolated poly alpha-1,6-glucan ether product can be dried using any method known in the art, such as vacuum drying, air drying, or freeze drying.

Any of the above etherification reactions can be repeated using a poly alpha-1,6-glucan ether product as the starting material for further modification. This approach may be suitable for increasing the DoS of a positively charged organic group, and/or adding one or more different positively charged organic groups to the ether product. Also, this approach may be suitable for adding one or more organic groups that are not positively charged, such as an alkyl group (e.g., methyl, ethyl, propyl, butyl) and/or a hydroxyalkyl group (e.g., hydroxyethyl, hydroxypropyl, hydroxybutyl). Any of the above etherification agents, but without the substitution with a positively charged group, can be used for this purpose.

As described above, materials derived from sustainable/renewable feedstock materials are often desirable. Similarly, biodegradable materials may also be preferred. For example, biodegradable cationic poly alpha-1,6-glucan ether compounds are preferred over non-biodegradable materials from an environmental footprint perspective. The biodegradability of a material can be evaluated by methods known in the art, for example as disclosed in the Biodegradability Test Method section herein below. The cationic poly alpha-1,6-glucan ether compound may be characterized by a biodegradability as determined by the Biodegradability Test Method below (i.e., Carbon Dioxide Evolution Test Method - OECD Guideline 301B) of at least 10% on the 90^{th} day of the test duration. The cationic poly alpha-1,6-glucan ether compound may be characterized by a biodegradability, as determined by the Biodegradability Test Method below, of at least 5%, 10%, 15%, 20%, 25%, 30%, 35%, 40%, 45%, 50%, 55%, 60%, 65%, 70%, 75%, or 80%, or any value between 5% and 80%, on the 90^{th} day of the test duration. The cationic poly alpha-1,6-glucan ether compound may be characterized by a biodegradability, as determined by the Biodegradability Test Method below, of at least 5%, 10%, 15%, 20%, 25%, 30%, 35%, 40%, 45%, 50%, 55%, or 60%, or any value between 5% and 60%, on the 60^{th} day of the test duration. Without wishing to be bound by theory, it is believed that the biodegradability profile of the presently described materials may be affected by the degree of substitution, the molecular weight, the degree of branching, and/or the solubility of the material. For example, it is believed that relatively lower degrees of substitution (e.g., lower cationic charge density) and/or increased solubility will be associated with higher degrees of biodegradability.

Wherein the water-soluble unit dose article is a multi-compartment unit dose article, the cationic poly alpha-1,6-glucan ether compound may be comprised in any compartment, or any combination of compartments, or even in each compartment.

### Method of making

Those skilled in the art will be aware of known methods and techniques to make the water-soluble unit dose article, liquid laundry treatment composition and ingredients thereof.

### Method of use

A further aspect of the present invention is a process for washing fabrics comprising the steps of diluting a water-soluble unit dose article according to the present invention in water by a factor of between 200 and 3000 fold to create a wash liquor and contacting fabrics to be washed with said wash liquor. Preferably the wash liquor comprises between 5L and 75L, preferably between 7L and 40L, more preferably between 10L and 20L of water. Preferably, the wash liquor is at a temperature of between 5°C and 90°C, preferably between 10°C and 60°C, more preferably between 12°C and 45°C, most preferably between 15°C and 40°C. Preferably, washing the fabrics in the wash liquor takes between 5 minutes and 50 minutes, preferably between 5 minutes and 40 minutes, more preferably between 5 minutes and 30 minutes, even more preferably between 5 minutes and 20 minutes, most preferably between 6 minutes and 18 minutes to complete. Preferably, the wash liquor comprises between 1kg and 20 kg, preferably between 3kg and 15kg, most preferably between 5 and 10 kg of fabrics. The wash liquor may comprise water of any hardness preferably varying between 0 gpg to 40gpg.

The dimensions and values disclosed herein are not to be understood as being strictly limited to the exact numerical values recited. Instead, unless otherwise specified, each such dimension is intended to mean both the recited value and a functionally equivalent range surrounding that value. For example, a dimension disclosed as "40 mm" is intended to mean "about 40 mm."

### EXAMPLES

The impact of single variable addition of a cationically modified poly alpha-1,6-glucan ether compound according to the invention on top of a water soluble unit dose liquid laundry formulation has been assessed for delivering a fabric care benefit, as well as its potential to mitigate the freshness negative typically observed in presence of cationic hydroxyethyl cellulose and polyvinyl alcohol. The performance impact has been assessed following the test methods described herein.

### Example 1 : Fabric freshness impact

The fabric freshness impact of single variable addition of a cationically modified poly alpha-1,6-glucan ether compound according to the invention as well as of a cationically modified hydroxyethyl cellulose on top of a liquid laundry detergent base (composition : see table 1) suitable for use in soluble unit dose laundry formulations has been assessed both in presence and absence of a water soluble polyvinylalcohol film following the test method described herein.

### Test method :

### Treatment of test fabrics:

The method of treating a fabric includes the use of a commercial washing machine, such as a Miele Honeycomb Care W1724, or other similar machine using standard machine settings (Cotton Short cycle at 40C, 1:38 long total cycle) followed by 24 hours line drying in a constant temperature / humidity room (70°F / 50% rH). Fabrics are treated multiple cycles (3) prior to analysis. Fabric composition in the machine consists of test fabrics and standard ballast comprising of a mixture of polyester, polycotton, and cotton, totaling 5.5 pounds. Within each treatment cycle the polymer and detergent treatments are delivered to the drum of the machine at the designated level (26.65 g detergent base, 1g PVA film, 10-20 ppm polymer in wash solution), prior to the fabrics. After the wash cycle the fabrics are exposed to one or more rinse cycles.

### Freshness grading

One of the test designs recommended by ASTM (E1958) for finding differences in measurable attributes is using a trained descriptive analysis panel. Fourteen validated external (non-employee) descriptive analysis panelists who grade on perfume intensity were trained on how to grade the fabrics for dry fabric perfume intensity using their typical 0-100 scale (the higher the better). The protocols of grading were pre-rub (smelling different portions of the fabric) & post-rub (rubbing a fabric together 5 times and smelling once). All samples were labeled with a blinded 3-digit code, and presentation order was randomized. Three replications were placed in this test and test gradings were averaged.

Starting materials :
- Table 1 describes a first liquid laundry base detergent composition.
- cationically modified poly alpha-1,6-glucan ether compound (MW 185M, cationic degree of substitution 0.07%, degree of branching 5%), as received from DuPont company.
- Cationically modified hydroxyethyl cellulose, Polyquaternium 10 (MW 300-500M, low cationic charge density e.g <1% nitrogen), as received from Dow company
- Water soluble film : polyvinylalcohol homopolymer / anionic polyvinylalcohol copolymer blend, as received from the MonoSol company

**Table 1 : Liquid laundry base composition 1 :**

| Ingredients | Active level (100% active basis) |
|---|---|
| Nonionic surfactant (Neodol 24-7) | 3.1 |
| Anionic surfactant (MEA-C24 HAE₃S) | 8.9 |
| Anionic surfactant (HLAS) | 27.0 |
| Citric Acid | 0.7 |
| TPK Fatty Acid | 11.2 |
| Enzymes | 0.7 |
| Ethoxylated polyethyleneimine (PEI₆₀₀EO₂₀ - Lutensol FP620 ex BASF) | 1.5 |
| Zwitterionic polyamine (Lutensit Z96 ex BASF) | 1.5 |
| HEDP chelant | 0.7 |
| Brightener 49 | 0.3 |
| 1,2-Propanediol | 15.8 |
| Glycerol | 4.9 |
| Monoethanolamine | 8.2 |
| Potassium Sulfite (K₂SO₃) | 0.1 |
| Hydrogenated Castor Oil | 0.1 |
| Perfume (including free perfume and perfume capsules) | 3.8 |
| Water | 10.4 |
| Minors | Balance to 100 |
| pH | 7.4 |

### Test results :

Table 2 summarizes the absolute pre- and post-rub perfume expert gradings as well as the single variable freshness loss effect of polyvinylalcohol addition, for nil polymer and cationic hydroxyethyl cellulose comparative polymer references outside the scope of the invention, as well as for the examples comprising the cationic polyglucan according to the invention. The data clearly show the cationic polyglucan according to the invention partially mitigating the negative polyvinylalcohol driven freshness impact observed in the nil polymer and cationic hydroxyethyl cellulose comprising samples (relative % PVA impact values). Beyond, amongst the polyvinylalcohol film comprising samples, inherent for water soluble unit dose articles, single variable addition of cationic polyglucan (Inventive example 1) to a nil polymer reference (Comparative example 1) does not negatively impact fabric freshness performance, contrary to single variable addition of cationic hydroxyethyl cellulose (Comparative example 3) where a clear fabric freshness performance compromise is observed.

**Table 2 : Fabric Freshness performance**

| | Comparative Example 1 | Comparative Example 2 | % PVA impact | | Comparative Example 3 | Comparative Example 4 | % PVA impact | | Inventive Example 1 | Comparative Example 5 | % PVA impact |
|---|---|---|---|---|---|---|---|---|---|---|---|
| | nil polymer, with PVA film | nil polymer, nil PVA film | | | 10ppm CatHEC, with PVA film | 10 ppm CatHEC, nil PVA film | | | 20ppm cationic polyglucan , with PVA film | 20ppm cationic polyglucan , nil PVA film | |
| Pre-rub Perfume | 33.4 | 40.3 | 17.2 % | | 30.9 | 35.4 | 12.7 % | | 34.1 | 37.5 | 9.0% |
| Post-rub Perfume | 41.4 | 46.0 | 10.0 % | | 35.7 | 40.6 | 12.0 % | | 41.9 | 43.3 | 3.2% |

### Example 2. Fabric Retention Performance in a Soluble Unit Dose Detergent Formulation

The fabric retention impact of single variable addition of a cationically modified poly alpha-1,6-glucan ether compound according to the invention as well as of a cationically modified hydroxyethyl cellulose on top of a liquid laundry detergent base (composition : see table 3) suitable for use in soluble unit dose laundry formulations has been assessed following the test method described herein.

### Treatment of test fabrics:

The method of treating a fabric includes the use of a commercial washing machine, such as a Miele Honeycomb Care W1724, or other similar machine using standard machine settings (Cotton Short cycle at 40C, 1:38 long total cycle) followed by 24 hours line drying in a constant temperature / humidity room (70°F / 50% rH). Fabrics are treated multiple cycles (3) prior to analysis. Fabric composition in the machine consists of test fabrics and standard ballast comprising of a mixture of polyester, polycotton, and cotton, totaling 5.5 pounds. Within each treatment cycle the polymer and detergent treatments are delivered to the drum of the machine at the designated level (26.65 g detergent base, 1g PVA film, 38 ppm polymer in wash solution), prior to the fabrics. After the wash cycle the fabrics are exposed to one or more rinse cycles.

### Secant Modulus Instron Method

The Secant Modulus is measured using a Tensile and Compression Tester Instrument, such as the Instron Model 5565 (Instron Corp., Norwood, Massachusetts, U.S.A.). The instrument is configured depending on the fabric type by selecting the following settings: the mode is Tensile Extension; the Waveform Shape is Triangle; the Maximum Strain is 10% for 479 Sanforized and 35% for 7422 Knitted, the Rate is 0.83mm/sec for 479 Sanforized and 2.5 mm/sec for 7422 Knitted, the number of Cycles is 4; and the Hold time is 15 seconds between cycles.
1. With scissors, cut serged edge of one entire side of each swatch in the warp direction and carefully peel off strings without stressing the fabric until an even edge is achieved.
2. Place a fabric press die that cuts strips 1" wide and at least 4" long parallel to the even edge and cut strips lengthwise in the warp direction.
3. Cut 3 strips of test fabric 479 Sanforized 100% cotton woven or test fabric 7422 50:50 polycotton knitted from 3 separate fabric swatches per treatment. Condition fabrics in a constant temperature (70°F) and humidity (50% RH) room for at least 6 hours before analysis.
4. Clamp the top and then the bottom of fabric strip into the 2.54cm grips on the tensile tester instrument with a 2.54 cm gap setting, loading a small amount of force (0.0.05N - 0.2N) on the sample.
5. Release bottom clamp and re-clamp sample during the hold cycle, loading 0.05N-0.2N of force on the sample removing the slack by again loading the same force.
6. When 4 hysteresis cycles have been completed for the sample, Secant Modulus is reported in megapascal (MPa). The final result is the average of the individual cycle 4 modulus results from all test strips for a given treatment on a given fabric type. The Secant Modulus reported is calculated at the Maximum Strain for each fabric type.

Starting materials :
- Table 3 describes a second liquid laundry base detergent composition.
- cationically modified poly alpha-1,6-glucan ether compounds: see table 4, as received from DuPont company.
- Cationically modified hydroxyethyl cellulose, Polyquaternium 10 (MW 300-500M, low cationic charge density e.g <1% nitrogen), as received from Dow company
- Water soluble film : polyvinylalcohol homopolymer / anionic polyvinylalcohol copolymer blend, as received from the MonoSol company

**Table 3. Liquid laundry base composition 2**

| | Wt% |
|---|---|
| Nonionic surfactant (Neodol 24 /7) | 2.9 |
| Anionic surfactant (HLAS) | 25.7 |
| Anionic surfactant (HC24 AE₃S) | 8.2 |
| Citric acid | 0.6 |
| TPK Fatty acid | 10.3 |
| Protease (76.3mg/g) | 0.05 |
| Amylase (29.26 mg/g) | 0.003 |
| Ethoxylated Polyethyleneimine (PEI₆₀₀ EO₂₀- Lutensol FP620 ex BASF) | 2.9 |
| Chelant (HEDP) | 0.8 |
| Brightener 49 (8.4% premix) | 0.3 |
| Antifoam | 0.3 |
| 1,2 Propanediol | 17.5 |
| Glycerol | 4.7 |
| Polypropylene glycol 400 | 1.1 |
| MEA (Monoethanolamine) | 8.9 |
| K₂SO₃ | 0.1 |
| Hydrogenated castor oil | 0.1 |
| Perfume | 2.4 |
| Encapsulated Perfume | 0.7 |
| Water | 10.3 |
| Minors | Balance to 100% |
| pH | 7.4 |

### Test Results:

Table 4 summarizes the resulting Secant Modulus measured following the test method described herein for a nil polymer reference product, as well as for detergent composition single variably comprising cationic polyglucan polymers according to the invention. The data clearly show single variable addition of the cationic polyglucan according to the invention resulting in a decreased secant modulus, indicating improved fabric retention benefit in line with the tested cationically modified hydroxyethylcellulose (Instron Secant Modulus of 3.5) accordingly. In polymers 1-3 listed below, the cationic group is a quaternized ammonium group substituted with three methyl groups (i.e., trimethyl ammonium quat). The cationic groups are linked to the ether group (and thus to the glucan backbone) by a hydroxypropyl group, but any suitable alkyl group or other hydroxyalkyl group could be used to link accordingly.

Table 4.

| **Example** | **PPM (polymer as 100% active)** | **Polymer characteristics** | | | **Instron Secant Modulus (7422)** |
|---|---|---|---|---|---|
| | | **Backbone MW (kDa)** | **Cationic DoS** | **Degree of Branching** | |
| Nil polymer | 0 | - | - | - | 7.2 |
| Polymer 1 | 38 | 185 | 0.15 | 5% | 3.4 |
| Polymer 2 | 38 | 185 | 0.38 | 5% | 4.8 |
| Polymer 3 | 38 | 200 | 0.19 | 10% | 4.6 |

In summary, single variable addition of cationic polyglucan polymers according to the invention to a water soluble unit dose liquid detergent composition results in improved fabric care benefits while mitigating negative freshness benefits as observed for alternative cationic polymer fabric care technologies such as cationically modified hydroxyethylcellulose and polyvinylalcohol water soluble film technology.

### Example 3. Fabric Retention Performance in different Soluble Unit Dose Detergent Formulation

The fabric retention impact of single variable addition of a cationically modified poly alpha-1,6-glucan ether compound according to the invention on top of a liquid laundry detergent base (composition : see table 3) suitable for use in soluble unit dose laundry formulations has been assessed following the test method described herein.

### Treatment of test fabrics:

The method of treating a fabric includes the use of a commercial washing machine, such as a Miele Honeycomb Care W1724, or other similar machine using standard machine settings (Cotton Short cycle at 40C, 1:38 long total cycle) followed by tumbling dry in a Miele T640 on cotton normal cycle. Fabrics are treated multiple cycles (6) prior to analysis. Fabric composition in the machine consists of test fabrics and standard ballast comprising of a mixture of polyester, polycotton, and cotton, totaling 5.5 pounds. Within each treatment cycle the polymer and detergent treatments are delivered to the drum of the machine at the designated level (26.01 g detergent base, 0.67g PVA film, 20 ppm polymer in wash solution), prior to the fabrics. After the wash cycle the fabrics are exposed to one or more rinse cycles.

### Secant Modulus Instron Method

The Secant Modulus is measured using a Tensile and Compression Tester Instrument, such as the Instron Model 3342 (Instron Corp., Norwood, Massachusetts, U.S.A.). The instrument is configured depending on the fabric type by selecting the following settings: the mode is Tensile Extension; the Waveform Shape is Triangle; the Maximum Strain is 10% for 479 Sanforized and 35% for 7422 Knitted, the Rate is 0.83mm/sec for 479 Sanforized and 2.5 mm/sec for 7422 Knitted, the number of Cycles is 4; and the Hold time is 15 seconds between cycles.
1. Place a fabric press die that cuts strips 1" wide and at least 4" long parallel to the even edge and cut strips lengthwise in the warp direction.
2. Cut 3 strips of test fabric 479 Sanforized 100% cotton woven or test fabric 7422 50:50 polycotton knitted from 3 separate fabric swatches per treatment. Condition fabrics in a constant temperature (70°F) and humidity (50% RH) room for at least 6 hours before analysis.
3. Clamp the top and then the bottom of fabric strip into the 2.54cm grips on the tensile tester instrument with a 2.54 cm gap setting, loading a small amount of force (0.05N - 0.2N) on the sample.
4. Release bottom clamp and re-clamp sample during the hold cycle, loading 0.05N-0.2N of force on the sample removing the slack by again loading the same force.
5. When 4 hysteresis cycles have been completed for the sample, Secant Modulus is reported in megapascal (MPa). The final result is the average of the individual cycle 4 modulus results from all test strips for a given treatment on a given fabric type. The Secant Modulus reported is calculated at the Maximum Strain for each fabric type.

Starting materials :
- Table 3 describes a second liquid laundry base detergent composition.
- cationically modified poly alpha-1,6-glucan ether compounds: see table 4, as received from DuPont company.
- Water soluble film : polyvinylalcohol homopolymer / anionic polyvinylalcohol copolymer blend, as received from the MonoSol company

**Table 5. Liquid laundry base composition**

| Active_Name | Composition 3 | Composition 4 | Composition 5 |
|---|---|---|---|
| | %wt | %wt | %wt |
| Water | 10.4040% | 10.3330% | 10.3217% |
| Citric Acid | 0.6511% | 0.6511% | 0.6511% |
| 1,2 Propanediol | 15.7513% | 19.7004% | 20.3015% |
| Monoethanolamine (MEA) | 8.2431% | 3.6796% | 3.8491% |
| Glycerine | 4.9576% | 4.9576% | 4.9576% |
| Chelant (HEDP) | 0.6905% | 0.6905% | 0.6905% |
| Potassium Sulfite (K2SO3) | 0.3986% | 0.3986% | 0.3986% |
| Nonionic surfactant (NI 24-7) | 3.0219% | 3.0219% | 21.1664% |
| Sulfuric Acid | 0.2789% | 0.1370% | 0.1144% |
| Benzene, C10-13-Alkyl Derivs. | 0.4184% | 0.2055% | 0.1717% |
| Anionic surfactant (HLAS) | 27.0578% | 13.2885% | 11.1003% |
| Sodium Chloride (NaCl) | 0.0161% | 0.0161% | 0.0161% |
| Brightener 49 | 0.2896% | 0.2896% | 0.2896% |
| TPK Fatty Acid | 11.2200% | 11.6039% | 11.4000% |
| MEA-C24 HAE3 S | 8.9406% | 23.0763% | 6.9519% |
| Alcohols, C12-16, ethoxylated (n=3) | 0.1834% | 0.4734% | 0.1426% |
| zwitterionic polyamine¹ | 1.4799% | 1.4799% | 1.4799% |
| Ethoxylated Polyethyleneimine (PEI₆₀₀ EO₂₀- Lutensol FP620 ex BASF) | 1.4799% | 1.4799% | 1.4799% |
| Magnesium Chloride (MgCl2) | 0.1320% | 0.1320% | 0.1320% |
| Sodium Formate (HCOONa) | 0.0573% | 0.0573% | 0.0573% |
| Encapsulated perfume | 0.8400% | 0.8400% | 0.8400% |
| Sorbitol | 0.0244% | 0.0244% | 0.0244% |
| Perfume | 3.3179% | 3.3179% | 3.3179% |
| Sodium Hydroxide (NaOH) | 0.0001% | 0.0001% | 0.0001% |
| HCO | 0.1440% | 0.1440% | 0.1440% |
| Benzisothiazolinone | 0.0004% | 0.0004% | 0.0004% |
| Dipropylene Glycol | 0.0011% | 0.0011% | 0.0011% |
| Minors | Balance to 100% | Balance to 100% | Balance to 100% |

| | | | |
|---|---|---|---|
| ¹ Lutensit Z96 (zwitterionic polyamine ex BASF - zwitterionic hexamethylene diamine according to below formula : 100% quaternized and about 40% of the polyethoxy (EO24) groups sulfonated). | | | |

### Test Results:

Table 6 summarizes the resulting Secant Modulus for knitted cotton 7422 measured following the test method described herein for a nil polymer reference product, as well as for detergent composition single variably comprising cationic polyglucan polymers according to the invention. The data clearly show single variable addition of the cationic polyglucan according to the invention resulting in a decreased secant modulus, indicating improved fabric retention benefit. In polymers 4-5 listed below, the cationic group is a quaternized ammonium group substituted with three methyl groups (i.e., trimethyl ammonium quat). The cationic groups are linked to the ether group (and thus to the glucan backbone) by a hydroxypropyl group, but any suitable alkyl group or other hydroxyalkyl group could be used to link accordingly. The data also suggest that inventive polymers show bigger impact on reducing secant modulus in a composition 4 and composition 5, which have higher AES-to-LAS ratio, or high nonionic surfactant-to-LAS ratio

**Table 6.**

| | **Example** | **PPM (polymer as 100% active)** | **Polymer characteristics** | | | **Instron Secant Modulus (7422)** | **Instron Secant Modulus (7422) vs Nil polymer (%)** |
|---|---|---|---|---|---|---|---|
| Composition | | | **Backbone MW (kDa)** | **Cationic DoS** | **Degree of Branching** | | |
| Composition 3 | Nil polymer | 0 | - | - | - | 9.3 | 100% |
| Composition 3 | Polymer 4 | 20 | 187 | 0.15 | 5% | 8.3 | 89% |
| Composition 3 | Polymer 5 | 20 | 187 | 0.07 | 5% | 7.5 | 81% |
| Composition 4 | Nil polymer | 0 | - | - | - | 9.2 | 100% |
| Composition 4 | Polymer 4 | 20 | 187 | 0.15 | 5% | 3.6 | 39% |
| Composition 4 | Polymer 5 | 20 | 187 | 0.07 | 5% | 5.0 | 53% |
| Composition 5 | Nil polymer | 0 | - | - | - | 9.6 | 100% |
| Composition 5 | Polymer 4 | 20 | 187 | 0.15 | 5% | 4.6 | 48% |
| Composition 5 | Polymer 5 | 20 | 187 | 0.07 | 5% | 6.7 | 70% |

It is clear from the data in Table 6 that cationic polyglucans according to the present invention deliver their performance across a wide range of surfactant formulations.

The dimensions and values disclosed herein are not to be understood as being strictly limited to the exact numerical values recited. Instead, unless otherwise specified, each such dimension is intended to mean both the recited value and a functionally equivalent range surrounding that value. For example, a dimension disclosed as "40 mm" is intended to mean "about 40 mm".

## Claims

1. A water-soluble unit dose article comprising a water-soluble film and a liquid laundry treatment composition;
wherein the water-soluble film comprises a polyvinylalcohol and is shaped to create an internal compartment, wherein the liquid laundry treatment composition is housed in said internal compartment; and
wherein the liquid laundry treatment composition comprises a cationically modified poly alpha-1,6-glucan ether compound,
wherein the treatment composition comprises from 0.01% to 10% by weight of the treatment composition, of the cationically modified poly alpha-1,6-glucan ether compound.

2. The water-soluble unit dose article according to claim 1, wherein the cationically modified poly alpha-1,6-glucan ether compound comprises a cationically modified poly alpha-1,6-glucan substituted with at least one positively charged organic group, wherein the poly alpha-1,6-glucan comprises a backbone of glucose monomer units wherein at least 65% of the glucose monomer units are linked via alpha-1,6-glycosidic linkages, and
wherein the cationically modified poly alpha-1,6-glucan ether compound has a degree of substitution of about 0.001 to about 3, preferably from 0.01 to 1.5, more preferably from 0.01 to 1.0, even more preferably from 0.01 to 0.8, most preferably from 0.03 to 0.7, or from 0.04 to 0.6, or from 0.05 to 0.5; and is **characterised by** at least one of the following i-iv;
i) a weight average degree of polymerization of at least 5, preferably 5 to 6000, more preferably from 50 to 5000, or from 100 to 4000, or from 250 to 3000, or from 500 to 2000, or from 750 to 1500, or from 1000 to 1400, or from 1100 to 1300;
ii) a weight average molecular weight of from 1000 to 500,000 daltons, preferably from 10,000 to 400,000 daltons, or from 40,000 to 300,000 daltons, or from 80,000 to about 300,000 or from about 100,000 to 250,000 daltons, or from 150,000 to 250,000 daltons, or from 180,000 to 225,000 daltons, or from 180,000 to 200,000 daltons;
iii) been derived from a poly alpha-1,6-glucan having a weight average molecular weight of from 900 to 450,000 daltons, preferably from 10,000 to 350,000 daltons, or from 50,000 to 350,000 daltons, or from 90,000 to 300,000 daltons, or from 125,000 to 250,000 daltons, or from 150,000 to 200,000 daltons, determined prior to substitution with the least one positively charged organic group;
iv) a mixture thereof.

3. The water-soluble unit dose article according to claim 1, wherein at least 3%, or at least 5%, preferably from 5% to 35%, more preferably from 5% to 30%, more preferably from 5% to 30%, more preferably from 5% to 25%, even more preferably from 5% to 20% of the backbone glucose monomer units have branches via alpha-1,2 and/or alpha-1,3-glycosidic linkages.

4. The water-soluble unit dose article according to any preceding claims, wherein the positively charged organic group comprises a substituted ammonium group, preferably a quaternary ammonium group, more preferably, wherein the quaternary ammonium group comprises at least one C₁ to C₁₈ alkyl group, even more preferably, wherein the quaternary ammonium group comprises at least one C₁ to C₄ alkyl group, most preferably wherein the quaternary ammonium group comprises two C₁ to C₄ alkyl groups or even three C₁ to C₄ alkyl groups.

5. The water-soluble unit dose article according to claim 4, wherein the quaternary ammonium group comprises at least one C₁₀ to C₁₆ alkyl group, preferably wherein the quaternary ammonium group comprises at least one C₁₀ to C₁₆ alkyl group and two C₁ to C₄ alkyl groups.

6. The water-soluble unit dose article according to claims 3-4 wherein the quaternary ammonium group comprises a trimethylammonium group.

7. The water-soluble unit dose article according to any preceding claims, wherein the positively charged organic group comprises a quaternary ammonium hydroxyalkyl group, preferably wherein the quaternary ammonium hydroxyalkyl group comprises a quaternary ammonium hydroxymethyl group, a quaternary ammonium hydroxyethyl group, a quaternary ammonium hydroxypropyl group, or a mixture thereof, more preferably, wherein the quaternary ammonium hydroxyalkyl group comprises a trimethylammonium hydroxyalkyl group, most preferably a trimethylammonium hydroxypropyl group.

8. The water-soluble unit dose article according to any preceding claims, wherein the cationically modified poly alpha-1,6-glucan comprises a backbone of glucose monomer units wherein at least 70%, or at least 75%, or at least 80%, or at least 90%, or at least 95% of the glucose monomer units are linked via alpha-1,6-glycosidic linkages.

9. The water-soluble unit dose article according to any preceding claims, wherein the treatment composition comprises from 0.3% to 3%, or from 0.5% to 2.0%, by weight of the treatment composition, of the cationically modified poly alpha-1,6-glucan ether compound.

10. The water-soluble unit dose article according to any preceding claims wherein the water-soluble film comprises a polyvinylalcohol homopolymer or a polyvinylalcohol copolymer, preferably a blend of polyvinylalcohol homopolymers and/or anionic polyvinylalcohol copolymers more preferably selected from sulphonated and carboxylated anionic polyvinylalcohol copolymers especially carboxylated anionic polyvinylalcohol copolymers, most preferably a blend of a polyvinylalcohol homopolymer and a carboxylated anionic polyvinylalcohol copolymer.

11. The water-soluble unit dose article according to any preceding claims, wherein the liquid laundry treatment composition comprises a non-soap surfactant, preferably wherein the liquid treatment composition comprises between 20% and 60%, preferably between 25% and 55%, more preferably between 30% and 50% by weight of the liquid laundry treatment composition of the non-soap surfactant, preferably wherein the non-soap surfactant is selected from anionic surfactants, non-ionic surfactants, cationic surfactants, amphoteric surfactants, zwitterionic surfactants, or a mixture thereof, preferably from anionic surfactants, non-ionic surfactants, or a mixture thereof, most preferably from anionic surfactants and non-ionic surfactants wherein the weight ratio of non-soap anionic surfactant to nonionic surfactant is from 1:1 to 20:1, from 1.5:1 to 17.5:1, from 2:1 to 15:1, or from 2.5:1 to 13:1.

12. The water-soluble unit dose article according to claim 11, wherein the non-soap anionic surfactant comprises linear alkyl benzene sulphonate, alkoxylated alkyl sulphate, or a mixture thereof, preferably wherein the non-soap anionic surfactant comprises linear alkyl benzene sulphonate and alkoxylated alkyl sulphate and wherein the weight ratio of linear alkylbenzene sulphonate to alkoxylated alkyl sulphate is from 1:2 to 9:1, preferably from 1:1 to 7:1, more preferably from 1:1 to 5:1, most preferably from 1:1 to 4:1.

13. The water-soluble unit dose article according to any preceding claims wherein the liquid laundry treatment composition comprises a perfume raw material.

14. The water-soluble unit dose article according to any preceding claims wherein the liquid laundry treatment composition comprises between 1% and 20%, preferably between 5% and 15% by weight of the liquid laundry detergent composition of water.

15. A process for washing fabrics comprising the steps of diluting a water-soluble unit dose article according to any preceding claims in water by a factor of between 200 and 3000 fold to create a wash liquor and contacting fabrics to be washed with said wash liquor.

## Patentansprüche

1. Wasserlöslicher Einheitsdosisartikel, umfassend eine wasserlösliche Folie und eine flüssige Wäschebehandlungszusammensetzung;
wobei die wasserlösliche Folie einen Polyvinylalkohol umfasst und so geformt ist, dass sie ein Innenfach bildet, wobei die flüssige Wäschebehandlungszusammensetzung in dem Innenfach untergebracht ist; und
wobei die flüssige Wäschebehandlungszusammensetzung eine kationisch modifizierte Poly-Alpha-1,6-Glucanether-Verbindung umfasst,
wobei die Behandlungszusammensetzung von 0,01 Gew.-% bis 10 Gew.-%, bezogen auf die Behandlungszusammensetzung, der kationisch modifizierten Poly-Alpha-1,6-Glucanether-Verbindung umfasst.

2. Wasserlöslicher Einheitsdosisartikel nach Anspruch 1, wobei die kationisch modifizierte Poly-Alpha-1,6-Glucanether-Verbindung ein kationisch modifiziertes Poly-Alpha-1,6-Glucan umfasst, das mit mindestens einer positiv geladenen organischen Gruppe substituiert ist, wobei das Poly-Alpha-1,6-Glucan ein Grundgerüst aus Glucosemonomereinheiten umfasst, wobei mindestens 65 % der Glucosemonomereinheiten über alpha-1,6-glycosidische Bindungen verknüpft sind, und
wobei die kationisch modifizierte Poly-Alpha-1,6-Glucanether-Verbindung einen Substitutionsgrad von etwa 0,001 bis etwa 3 aufweist, vorzugsweise von 0,01 bis 1,5, mehr bevorzugt von 0,01 bis 1,0, noch mehr bevorzugt von 0,01 bis 0,8, am meisten bevorzugt von 0,03 bis 0,7 oder von 0,04 bis 0,6 oder von 0,05 bis 0,5; und **gekennzeichnet ist durch** mindestens eines der folgenden i bis iv;
i) einen gewichtsdurchschnittlichen Polymerisationsgrad von mindestens 5, vorzugsweise 5 bis 6000, mehr bevorzugt von 50 bis 5000 oder von 100 bis 4000 oder von 250 bis 3000 oder von 500 bis 2000 oder von 750 bis 1500 oder von 1000 bis 1400 oder von 1100 bis 1300;
ii) ein gewichtsdurchschnittliches Molekulargewicht (Gewichtsmittel) von 1000 bis 500.000 Dalton, vorzugsweise von 10.000 bis 400.000 Dalton, oder von 40.000 bis 300.000 Dalton, oder von 80.000 bis etwa 300.000 oder von etwa 100.000 bis 250.000 Dalton, oder von 150.000 bis 250.000 Dalton, oder von 180.000 bis 225.000 Dalton, oder von 180.000 bis 200.000 Dalton;
iii) abgeleitet aus einem Poly-Alpha-1,6-Glucan mit einem gewichtsmittleren Molekulargewicht (Gewichtsmittel) von 900 bis 450.000 Dalton, vorzugsweise von 10.000 bis 350.000 Dalton oder von 50.000 bis 350.000 Dalton oder von 90.000 bis 300.000 Dalton oder von 125.000 bis 250.000 Dalton oder von 150.000 bis 200.000 Dalton, bestimmt vor der Substitution mit der mindestens einen positiv geladenen organischen Gruppe;
iv) eine Mischung davon.

3. Wasserlöslicher Einheitsdosisartikel nach Anspruch 1, wobei mindestens 3 % oder mindestens 5 %, vorzugsweise von 5 % bis 35 %, mehr bevorzugt von 5 % bis 30 %, mehr bevorzugt von 5 % bis 30 %, mehr bevorzugt von 5 % bis 25 %, noch mehr bevorzugt von 5 % bis 20 % der Glucosemonomereinheiten des Grundgerüsts Verzweigungen über Alpha-1,2- und/oder alpha-1,3-glycosidische Bindungen aufweisen.

4. Wasserlöslicher Einheitsdosisartikel nach einem der vorstehenden Ansprüche, wobei die positiv geladene organische Gruppe eine substituierte Ammoniumgruppe umfasst, vorzugsweise eine quartäre Ammoniumgruppe, wobei mehr bevorzugt die quartäre Ammoniumgruppe mindestens eine C₁- bis C₁₈-Alkylgruppe, wobei noch mehr bevorzugt die quartäre Ammoniumgruppe mindestens eine C₁- bis C₄-Alkylgruppe, wobei am meisten bevorzugt die quartäre Ammoniumgruppe zwei C₁- bis C₄-Alkylgruppen oder sogar drei C₁- bis C₄-Alkylgruppen umfasst.

5. Wasserlöslicher Einheitsdosisartikel nach Anspruch 4, wobei die quartäre Ammoniumgruppe mindestens eine C₁₀- bis C₁₆-Alkylgruppe, wobei die quartäre Ammoniumgruppe vorzugsweise mindestens eine C₁₀- bis C₁₆-Alkylgruppe und zwei C₁- bis C₄-Alkylgruppen umfasst.

6. Wasserlöslicher Einheitsdosisartikel nach Anspruch 3 bis 4, wobei die quartäre Ammoniumgruppe eine Trimethylammoniumgruppe umfasst.

7. Wasserlöslicher Einheitsdosisartikel nach einem der vorstehenden Ansprüche, wobei die positiv geladene organische Gruppe eine quartäre Ammoniumhydroxyalkylgruppe umfasst, vorzugsweise wobei die quartäre Ammoniumhydroxyalkylgruppe eine quartäre Ammoniumhydroxymethylgruppe, eine quartäre Ammoniumhydroxyethylgruppe, eine quartäre Ammoniumhydroxypropylgruppe oder eine Mischung davon umfasst, wobei mehr bevorzugt die quartäre Ammoniumhydroxyalkylgruppe eine Trimethylammoniumhydroxyalkylgruppe umfasst, am meisten bevorzugt eine Trimethylammoniumhydroxypropylgruppe.

8. Wasserlöslicher Einheitsdosisartikel nach einem der vorstehenden Ansprüche, wobei das kationisch modifizierte Poly-Alpha-1,6-Glucan ein Grundgerüst aus Glucosemonomereinheiten umfasst, wobei mindestens 70 %, oder mindestens 75 %, oder mindestens 80 %, oder mindestens 90 %, oder mindestens 95 % der Glucosemonomereinheiten über alpha-1,6-glycosidische Bindungen verknüpft sind.

9. Wasserlöslicher Einheitsdosisartikel nach einem der vorstehenden Ansprüche, wobei die Behandlungszusammensetzung von 0,3 Gew.% bis 3 Gew.-% oder von 0,5 Gew.-% bis 2,0 Gew.-%, bezogen auf die Behandlungszusammensetzung, der kationisch modifizierten Poly-Alpha-1,6-Glucanether-Verbindung umfasst.

10. Wasserlöslicher Einheitsdosisartikel nach einem der vorstehenden Ansprüche, wobei die wasserlösliche Folie ein Polyvinylalkoholhomopolymer oder ein Polyvinylalkoholcopolymer umfasst, vorzugsweise ein Gemisch aus Polyvinylalkoholhomopolymeren und/oder anionischen Polyvinylalkoholcopolymeren, mehr bevorzugt ausgewählt aus sulfonierten und carboxylierten anionischen Polyvinylalkoholcopolymeren, insbesondere carboxylierten anionischen Polyvinylalkoholcopolymeren, am meisten bevorzugt ein Gemisch aus einem Polyvinylalkoholhomopolymer und einem carboxylierten anionischen Polyvinylalkoholcopolymer.

11. Wasserlöslicher Einheitsdosisartikel nach einem der vorstehenden Ansprüche, wobei die flüssige Wäschebehandlungszusammensetzung ein seifenfreies Tensid umfasst, wobei die flüssige Behandlungszusammensetzung vorzugsweise zwischen 20 und 60 Gew.-%, vorzugsweise zwischen 25 und 55 Gew.-%, mehr bevorzugt zwischen 30 und 50 Gew.-%, bezogen auf die flüssige Wäschebehandlungszusammensetzung des seifenfreien Tensids, umfasst, wobei das seifenfreie Tensid vorzugsweise ausgewählt ist aus anionischen Tensiden, nichtionischen Tensiden, kationischen Tensiden, amphoteren Tensiden, zwitterionischen Tensiden oder einer Mischung davon, vorzugsweise aus anionischen Tensiden, nichtionischen Tensiden oder einer Mischung davon, am meisten bevorzugt aus anionischen Tensiden und nichtionischen Tensiden, wobei das Gewichtsverhältnis von seifenfreiem anionischem Tensid zu nichtionischem Tensid von 1:1 bis 20:1, von 1,5:1 bis 17,5:1, von 2:1 bis 15:1 oder von 2,5:1 bis 13:1 beträgt.

12. Wasserlöslicher Einheitsdosisartikel nach Anspruch 11, wobei das seifenfreie anionische Tensid lineares Alkylbenzolsulfonat, alkoxyliertes Alkylsulfat oder einer Mischung davon umfasst, vorzugsweise wobei das seifenfreie anionische Tensid lineares Alkylbenzolsulfonat und alkoxyliertes Alkylsulfat umfasst und wobei das Gewichtsverhältnis von linearem Alkylbenzolsulfonat zu alkoxyliertem Alkylsulfat von 1:2 bis 9:1, vorzugsweise von 1:1 bis 7:1, mehr bevorzugt von 1:1 bis 5:1, am meisten bevorzugt von 1:1 bis 4:1 beträgt.

13. Wasserlöslicher Einheitsdosisartikel nach einem der vorstehenden Ansprüche, wobei die flüssige Wäschebehandlungszusammensetzung ein Duftstoffrohmaterial umfasst.

14. Wasserlöslicher Einheitsdosisartikel nach einem der vorstehenden Ansprüche, wobei die flüssige Wäschebehandlungszusammensetzung zu zwischen 1 Gew.-% und 20 Gew.-%, vorzugsweise zwischen 5 Gew.-% und 15 Gew.-%, bezogen auf die flüssige Wäschewaschmittelzusammensetzung, Wasser umfasst.

15. Verfahren zum Waschen von Stoff, umfassend die Schritte des Verdünnens eines wasserlöslichen Einheitsdosisartikels nach einem der vorstehenden Ansprüche in Wasser um einen Faktor zwischen dem 200- bis 3000-Fachen, um eine Waschflotte zu bilden, und des Inkontaktbringens des Stoffes mit der Waschflotte.

## Revendications

1. Article en dose unitaire hydrosoluble comprenant un film hydrosoluble et une composition liquide de traitement du linge ;
dans lequel le film hydrosoluble comprend un alcool polyvinylique et est façonné de manière à créer un compartiment interne, dans lequel la composition liquide de traitement du linge est logée dans ledit compartiment interne ; et
dans lequel la composition liquide de traitement du linge comprend un composé éther de poly alpha-1,6-glucane à modification cationique,
dans lequel la composition de traitement comprend de 0,01 % à 10 % en poids de la composition de traitement, du composé éther de poly alpha-1,6-glucane à modification cationique.

2. Article en dose unitaire hydrosoluble selon la revendication 1, dans lequel le composé éther de poly alpha-1,6-glucane à modification cationique comprend un poly alpha-1,6-glucane à modification cationique substitué par au moins un groupe organique chargé positivement, dans lequel le poly alpha-1,6-glucane comprend un squelette de motifs monomères de glucose dans lequel au moins 65 % des motifs monomères de glucose sont liés par des liaisons alpha-1,6-glycosidiques, et
dans lequel le composé éther de poly alpha-1,6-glucane à modification cationique a un degré de substitution d'environ 0,001 à environ 3, de préférence de 0,01 à 1,5, plus préférablement de 0,01 à 1,0, encore plus préférablement de 0,01 à 0,8, le plus préférablement de 0,03 à 0,7, ou de 0,04 à 0,6, ou de 0,05 à 0,5 ; et est **caractérisé par** au moins l'une des caractéristiques i-iv suivantes ;
i) un degré de polymérisation moyen en poids d'au moins 5, de préférence de 5 à 6 000, plus préférablement de 50 à 5 000, ou de 100 à 4 000, ou de 250 à 3 000, ou de 500 à 2 000, ou de 750 à 1 500, ou de 1 000 à 1 400, ou de 1 100 à 1 300 ;
ii) une masse moléculaire moyenne en poids allant de 1 000 à 500 000 daltons, de préférence de 10 000 à 400 000 daltons, ou de 40 000 à 300 000 daltons, ou de 80 000 à environ 300 000, ou d'environ 100 000 à 250 000 daltons, ou de 150 000 à 250 000 daltons, ou de 180 000 à 225 000 daltons, ou de 180 000 à 200 000 daltons ;
iii) être dérivé d'un poly alpha-1,6-glucane ayant une masse moléculaire moyenne en poids allant de 900 à 450 000 daltons, de préférence de 10 000 à 350 000 daltons, ou de 50 000 à 350 000 daltons, ou de 90 000 à 300 000 daltons, ou de 125 000 à 250 000 daltons, ou de 150 000 à 200 000 daltons, déterminé avant la substitution par l'au moins un groupe organique chargé positivement ;
iv) un mélange de celles-ci.

3. Article en dose unitaire hydrosoluble selon la revendication 1, dans lequel au moins 3 %, ou au moins 5 %, de préférence de 5 % à 35 %, plus préférablement de 5 % à 30 %, plus préférablement de 5 % à 30 %, plus préférablement de 5 % à 25 %, encore plus préférablement de 5 % à 20 % des motifs monomères de glucose du squelette ont des ramifications par le biais de liaisons alpha-1,2 et/ou alpha-1,3-glycosidiques.

4. Article en dose unitaire hydrosoluble selon l'une quelconque des revendications précédentes, dans lequel le groupe organique chargé positivement comprend un groupe ammonium substitué, de préférence un groupe ammonium quaternaire, plus préférablement, dans lequel le groupe ammonium quaternaire comprend au moins un groupe alkyle en C₁ à C₁₈, encore plus préférablement, dans lequel le groupe ammonium quaternaire comprend au moins un groupe alkyle en C₁ à C₄, le plus préférablement dans lequel le groupe ammonium quaternaire comprend deux groupes alkyle en C₁ à C₄ ou même trois groupes alkyle en C₁ à C₄.

5. Article en dose unitaire hydrosoluble selon la revendication 4, dans lequel le groupe ammonium quaternaire comprend au moins un groupe alkyle en C₁₀ à C₁₆, de préférence dans lequel le groupe ammonium quaternaire comprend au moins un groupe alkyle en C₁₀ à C₁₆ et deux groupes alkyle en C₁ à C₄.

6. Article en dose unitaire hydrosoluble selon les revendications 3 à 4, dans lequel le groupe ammonium quaternaire comprend un groupe triméthylammonium.

7. Article en dose unitaire hydrosoluble selon l'une quelconque des revendications précédentes, dans lequel le groupe organique chargé positivement comprend un groupe hydroxyalkyle d'ammonium quaternaire, de préférence dans lequel le groupe hydroxyalkyle d'ammonium quaternaire comprend un groupe hydroxyméthyle d'ammonium quaternaire, un groupe hydroxyéthyle d'ammonium quaternaire, un groupe hydroxypropyle d'ammonium quaternaire, ou un mélange de ceux-ci, plus préférablement, dans lequel le groupe hydroxyalkyle d'ammonium quaternaire comprend un groupe hydroxyalkyle de triméthylammonium, le plus préférablement un groupe hydroxypropyle de triméthylammonium.

8. Article en dose unitaire hydrosoluble selon l'une quelconque des revendications précédentes, dans lequel le poly alpha-1,6-glucane à modification cationique comprend un squelette de motifs monomères de glucose dans lequel au moins 70 %, ou au moins 75 %, ou au moins 80 %, ou au moins 90 %, ou au moins 95 % des motifs monomères de glucose sont liés par le biais de liaisons alpha-1,6-glycosidiques.

9. Article en dose unitaire hydrosoluble selon l'une quelconque des revendications précédentes, dans lequel la composition de traitement comprend de 0,3 % à 3 %, ou de 0,5 % à 2,0 %, en poids de la composition de traitement, du composé éther de poly alpha-1,6-glucane à modification cationique.

10. Article en dose unitaire hydrosoluble selon l'une quelconque des revendications précédentes, dans lequel le film hydrosoluble comprend un homopolymère d'alcool polyvinylique ou un copolymère d'alcool polyvinylique, de préférence un mélange d'homopolymères d'alcool polyvinylique et/ou de copolymères d'alcool polyvinylique anioniques, choisis plus préférablement parmi des copolymères d'alcool polyvinylique anioniques sulfonés et carboxylés, notamment des copolymères d'alcool polyvinylique anioniques carboxylés, le plus préférablement un mélange d'un homopolymère d'alcool polyvinylique et d'un copolymère d'alcool polyvinylique anionique carboxylé.

11. Article en dose unitaire hydrosoluble selon l'une quelconque des revendications précédentes, dans lequel la composition liquide de traitement du linge comprend un agent tensioactif non-savon, de préférence dans lequel la composition liquide de traitement comprend entre 20 % et 60 %, de préférence entre 25 % et 55 %, plus préférablement entre 30 % et 50 %, en poids de la composition liquide de traitement du linge, de l'agent tensioactif non-savon, de préférence, dans lequel l'agent tensioactif non-savon est choisi parmi des agents tensioactifs anioniques, agents tensioactifs non ioniques, agents tensioactifs cationiques, agents tensioactifs amphotères, agents tensioactifs zwittérioniques, ou un mélange de ceux-ci, de préférence parmi des agents tensioactifs anioniques, agents tensioactifs non ioniques, ou un mélange de ceux-ci, le plus préférablement parmi des agents tensioactifs anioniques et agents tensioactifs non ioniques, dans lequel le rapport en poids entre agent tensioactif anionique et agent tensioactif non ionique non-savon va de 1:1 à 20:1, de 1,5:1 à 17,5:1, de 2:1 à 15:1, ou de 2,5:1 à 13:1.

12. Article en dose unitaire hydrosoluble selon la revendication 11, dans lequel l'agent tensioactif anionique non-savon comprend un sulfonate d'alkylbenzène linéaire, un sulfate d'alkyle alcoxylé, ou un mélange de ceux-ci, de préférence dans lequel l'agent tensioactif anionique non-savon comprend un sulfonate d'alkylbenzène linéaire et un sulfate d'alkyle alcoxylé et dans lequel le rapport en poids entre sulfonate d'alkylbenzène linéaire et sulfate d'alkyle alcoxylé va de 1:2 à 9:1, de préférence de 1:1 à 7:1, plus préférablement de 1:1 à 5:1 ; le plus préférablement de 1:1 à 4:1.

13. Article en dose unitaire hydrosoluble selon l'une quelconque des revendications précédentes, dans lequel la composition liquide de traitement du linge comprend une matière première de parfum.

14. Article en dose unitaire hydrosoluble selon l'une quelconque des revendications précédentes, dans lequel la composition liquide de traitement du linge comprend entre 1 % et 20 %, de préférence entre 5 % et 15 %, en poids de la composition détergente liquide pour le lavage du linge, d'eau.

15. Procédé de lavage de tissus comprenant les étapes consistant à diluer un article en dose unitaire hydrosoluble selon l'une quelconque des revendications précédentes dans de l'eau par un facteur compris entre 200 et 3 000 fois afin de créer une liqueur de lavage, et à mettre en contact des tissus à laver avec ladite liqueur de lavage.
